



US011255051B2

(12) **United States Patent**  
**Calewarts et al.**

(10) **Patent No.:** **US 11,255,051 B2**  
(45) **Date of Patent:** **Feb. 22, 2022**

(54) **FIBROUS SHEET WITH IMPROVED PROPERTIES**

(71) Applicant: **KIMBERLY-CLARK WORLDWIDE, INC.**, Neenah, WI (US)

(72) Inventors: **Deborah J. Calewarts**, Winneconne, WI (US); **Jian Qin**, Appleton, WI (US); **Charles W. Colman**, Marietta, GA (US); **Cathleen M. Uttecht**, Menasha, WI (US); **Donald E. Waldroup**, Roswell, GA (US); **Francis P. Abuto**, Johns Creek, GA (US); **Jenny L. Day**, Woodstock, GA (US); **Stephen M. Lindsay**, Appleton, WI (US)

(73) Assignee: **Kimberly-Clark Worldwide, Inc.**, Neenah, WI (US)

(\*) Notice: Subject to any disclaimer, the term of this patent is extended or adjusted under 35 U.S.C. 154(b) by 0 days.

(21) Appl. No.: **16/767,614**

(22) PCT Filed: **Nov. 29, 2017**

(86) PCT No.: **PCT/US2017/063653**

§ 371 (c)(1),

(2) Date: **May 28, 2020**

(87) PCT Pub. No.: **WO2019/108172**

PCT Pub. Date: **Jun. 6, 2019**

(65) **Prior Publication Data**

US 2020/0370246 A1 Nov. 26, 2020

(51) **Int. Cl.**

**D21H 27/38** (2006.01)

**D04H 1/425** (2012.01)

**D04H 1/593** (2012.01)

**D21F 11/00** (2006.01)

**D21F 11/02** (2006.01)

**D21H 13/24** (2006.01)

**D21H 15/04** (2006.01)

**D21H 17/35** (2006.01)

**D21H 21/16** (2006.01)

**D04H 1/541** (2012.01)

**D04H 1/4374** (2012.01)

**D04H 1/559** (2012.01)

**D04H 1/732** (2012.01)

(52) **U.S. Cl.**

CPC ..... **D21H 27/38** (2013.01); **D04H 1/425**

(2013.01); **D04H 1/4374** (2013.01); **D04H**

**1/5412** (2020.05); **D04H 1/559** (2013.01);

**D04H 1/593** (2013.01); **D04H 1/732**

(2013.01); **D21F 11/002** (2013.01); **D21F**

**11/02** (2013.01); **D21H 13/24** (2013.01);

**D21H 15/04** (2013.01); **D21H 17/35**

(2013.01); **D21H 21/16** (2013.01); **D04H**

**1/5414** (2020.05); **D04H 1/5416** (2020.05);

**D10B 2321/021** (2013.01); **D10B 2331/04**

(2013.01)

(58) **Field of Classification Search**

CPC ..... D21H 17/36; D21H 27/38; D21H 13/24; D21H 15/04; D21H 17/35; D21H 21/16; D21H 21/56; D21F 11/002; D21F 11/02; B32B 2262/0276; B32B 2262/067; B32B 2262/14; B32B 29/007; D10B 2321/021; D10B 2331/04; D04H 1/593; D04H 1/425; D04H 1/4374; D04H 1/559; D04H 1/732; D04H 1/541; D04H 1/5412

See application file for complete search history.

(56) **References Cited**

U.S. PATENT DOCUMENTS

|             |         |                  |
|-------------|---------|------------------|
| 2,105,711 A | 1/1938  | Weathered        |
| 2,791,523 A | 5/1957  | Schoen           |
| 3,007,840 A | 11/1961 | Wilcox           |
| 3,506,538 A | 4/1970  | Friedberg et al. |

(Continued)

FOREIGN PATENT DOCUMENTS

|    |           |         |
|----|-----------|---------|
| AT | 517303 A1 | 12/2016 |
| AT | 519414 A2 | 6/2018  |

(Continued)

OTHER PUBLICATIONS

Hubbe et al., in "Wet-Laid Nonwovens Manufacture Chemical Approaches Using Synthetic and Cellulosic Fibers" BioResources 11(2) pp. 5500-5552. (Year: 2016).\*

(Continued)

*Primary Examiner* — Jose A Fortuna

(74) *Attorney, Agent, or Firm* — Kimberly-Clark Worldwide, Inc.

(57) **ABSTRACT**

A method for producing a foam-formed multilayered substrate that includes producing an aqueous-based foam including at least 3% by weight non-straight synthetic binder fibers, wherein the non-straight synthetic binder fibers have an average length greater than 2 mm; forming together a wet sheet layer from the aqueous-based foam and a cellulosic fiber layer, wherein the cellulosic fiber layer includes at least 60 percent by weight cellulosic fibers; and drying the combined layers to obtain the foam-formed multilayer substrate. A multilayered substrate includes a first layer including at least 60 percent by weight non-straight synthetic binder fibers having an average length greater than 2 mm; and a second layer including at least 60 percent by weight cellulosic fiber, wherein the first layer is in a facing relationship with the second layer, and wherein the multilayered substrate has a wet/dry tensile ratio of at least 60%.

# US 11,255,051 B2

Page 2

---

| (56)                  | References Cited |                          |             |         |                  |  |
|-----------------------|------------------|--------------------------|-------------|---------|------------------|--|
| U.S. PATENT DOCUMENTS |                  |                          |             |         |                  |  |
| 3,542,640 A           | 11/1970          | Friedberg et al.         | 5,369,007 A | 11/1994 | Kidwell          |  |
| 3,615,975 A           | 10/1971          | Gillern et al.           | 5,372,766 A | 12/1994 | Roe              |  |
| 3,716,449 A           | 2/1973           | Gatward et al.           | 5,384,179 A | 1/1995  | Roe et al.       |  |
| 3,798,122 A           | 3/1974           | Appel                    | 5,387,207 A | 2/1995  | Dyer et al.      |  |
| 3,837,999 A           | 9/1974           | Chung                    | 5,393,379 A | 2/1995  | Parrinello       |  |
| 3,839,142 A           | 10/1974          | Clarke et al.            | 5,397,316 A | 3/1995  | LaVon et al.     |  |
| 3,871,952 A           | 3/1975           | Robertson                | 5,397,626 A | 3/1995  | Berg et al.      |  |
| 3,929,560 A           | 12/1975          | Holik et al.             | 5,409,572 A | 4/1995  | Kershaw et al.   |  |
| 3,938,782 A           | 2/1976           | Robertson                | 5,428,076 A | 6/1995  | Roe              |  |
| 3,966,540 A           | 6/1976           | Selander et al.          | 5,434,194 A | 7/1995  | Fujimoto et al.  |  |
| 4,007,083 A           | 2/1977           | Ring et al.              | 5,451,452 A | 9/1995  | Phan et al.      |  |
| 4,049,491 A           | 9/1977           | Brandon et al.           | 5,468,437 A | 11/1995 | Hall             |  |
| 4,062,721 A           | 12/1977          | Guyer et al.             | 5,506,046 A | 4/1996  | Andersen et al.  |  |
| 4,123,787 A           | 10/1978          | Leclerc du Sablon et al. | 5,506,277 A | 4/1996  | Griesbach        |  |
| 4,200,488 A           | 4/1980           | Brandon et al.           | 5,508,072 A | 4/1996  | Andersen et al.  |  |
| 4,285,767 A           | 8/1981           | Page                     | 5,533,244 A | 7/1996  | Wadzinski        |  |
| 4,288,475 A           | 9/1981           | Meeker                   | 5,536,264 A | 7/1996  | Hsueh et al.     |  |
| 4,299,655 A           | 11/1981          | Skaugen                  | 5,545,450 A | 8/1996  | Andersen et al.  |  |
| 4,394,930 A           | 7/1983           | Korpman                  | 5,549,589 A | 8/1996  | Homey et al.     |  |
| 4,415,388 A           | 11/1983          | Korpman                  | 5,550,167 A | 8/1996  | DesMarais        |  |
| 4,443,232 A           | 4/1984           | Kaiser                   | 5,560,878 A | 10/1996 | Dragoo et al.    |  |
| 4,443,297 A           | 4/1984           | Cheshire et al.          | 5,563,179 A | 10/1996 | Stone et al.     |  |
| 4,443,299 A           | 4/1984           | Cheshire et al.          | D375,633 S  | 11/1996 | Spanagel et al.  |  |
| 4,464,224 A           | 8/1984           | Matolcsy                 | 5,571,849 A | 11/1996 | DesMarais        |  |
| 4,478,615 A           | 10/1984          | Kaiser                   | 5,580,624 A | 12/1996 | Andersen et al.  |  |
| 4,483,976 A *         | 11/1984          | Yamamoto .....           | 5,582,670 A | 12/1996 | Andersen et al.  |  |
|                       |                  | D01F 6/86                | 5,585,432 A | 12/1996 | Lee et al.       |  |
|                       |                  | 528/275                  | 5,586,842 A | 12/1996 | Bae et al.       |  |
|                       |                  |                          | 5,599,334 A | 2/1997  | Johnston et al.  |  |
|                       |                  |                          | 5,612,385 A | 3/1997  | Ceaser et al.    |  |
|                       |                  |                          | D378,876 S  | 4/1997  | Spanagel et al.  |  |
| 4,498,956 A           | 2/1985           | Cheshire et al.          | 5,618,341 A | 4/1997  | Andersen et al.  |  |
| 4,543,156 A           | 9/1985           | Cheshire et al.          | 5,624,971 A | 4/1997  | Wilson           |  |
| 4,613,627 A           | 9/1986           | Sherman et al.           | 5,626,857 A | 5/1997  | Thimineur et al. |  |
| 4,655,950 A           | 4/1987           | Michalek                 | 5,631,053 A | 5/1997  | Andersen et al.  |  |
| 4,686,006 A           | 8/1987           | Cheshire et al.          | 5,632,737 A | 5/1997  | Stone et al.     |  |
| 4,734,321 A           | 3/1988           | Radvan et al.            | 5,633,291 A | 5/1997  | Dyer et al.      |  |
| 4,764,253 A           | 8/1988           | Cheshire et al.          | 5,649,409 A | 7/1997  | Gujer et al.     |  |
| 4,773,408 A           | 9/1988           | Cilento et al.           | 5,650,222 A | 7/1997  | DesMarais et al. |  |
| 4,773,409 A           | 9/1988           | Cilento et al.           | D381,810 S  | 8/1997  | Schultz et al.   |  |
| 4,778,477 A           | 10/1988          | Lauchenaier              | 5,658,603 A | 8/1997  | Andersen et al.  |  |
| 4,883,478 A           | 11/1989          | Lerailler et al.         | 5,660,900 A | 8/1997  | Andersen et al.  |  |
| 4,939,030 A           | 7/1990           | Tsuji et al.             | 5,660,903 A | 8/1997  | Andersen et al.  |  |
| 4,944,843 A           | 7/1990           | Wallace et al.           | 5,660,904 A | 8/1997  | Andersen et al.  |  |
| 4,948,007 A           | 8/1990           | Berg et al.              | 5,662,731 A | 9/1997  | Andersen et al.  |  |
| 4,952,448 A           | 8/1990           | Bullock et al.           | 5,665,442 A | 9/1997  | Andersen et al.  |  |
| 4,969,975 A           | 11/1990          | Biggs et al.             | 5,674,917 A | 10/1997 | Wilson           |  |
| 4,973,382 A           | 11/1990          | Kinn et al.              | 5,679,145 A | 10/1997 | Andersen et al.  |  |
| 4,985,467 A           | 1/1991           | Kelly et al.             | 5,679,218 A | 10/1997 | Vinson et al.    |  |
| 5,006,373 A           | 4/1991           | Woodmansee et al.        | 5,683,772 A | 11/1997 | Andersen et al.  |  |
| 5,008,306 A           | 4/1991           | Goguelin                 | 5,691,014 A | 11/1997 | Andersen et al.  |  |
| 5,013,405 A           | 5/1991           | Izard                    | 5,692,939 A | 12/1997 | DesMarais        |  |
| 5,064,653 A           | 11/1991          | Sessions et al.          | 5,693,403 A | 12/1997 | Brown et al.     |  |
| 5,065,752 A           | 11/1991          | Sessions et al.          | 5,695,607 A | 12/1997 | Oriaran et al.   |  |
| 5,073,416 A           | 12/1991          | Avakian et al.           | 5,702,571 A | 12/1997 | Kamps et al.     |  |
| 5,098,778 A           | 3/1992           | Minnick                  | 5,705,203 A | 1/1998  | Andersen et al.  |  |
| 5,102,501 A           | 4/1992           | Eber et al.              | 5,705,238 A | 1/1998  | Andersen et al.  |  |
| 5,134,959 A           | 8/1992           | Woodmansee et al.        | 5,705,239 A | 1/1998  | Andersen et al.  |  |
| 5,137,551 A           | 8/1992           | Ahrens et al.            | 5,705,242 A | 1/1998  | Andersen et al.  |  |
| 5,147,345 A           | 9/1992           | Young et al.             | 5,707,474 A | 1/1998  | Andersen et al.  |  |
| 5,153,058 A           | 10/1992          | Hall et al.              | 5,707,579 A | 1/1998  | Habelski et al.  |  |
| 5,164,045 A           | 11/1992          | Awofeso et al.           | 5,709,827 A | 1/1998  | Andersen et al.  |  |
| 5,178,729 A           | 1/1993           | Janda                    | 5,709,913 A | 1/1998  | Andersen et al.  |  |
| 5,196,090 A           | 3/1993           | Corbellini et al.        | D390,363 S  | 2/1998  | Baum et al.      |  |
| 5,200,035 A           | 4/1993           | Bhat et al.              | 5,713,881 A | 2/1998  | Rezai et al.     |  |
| 5,227,023 A           | 7/1993           | Pounder et al.           | 5,716,563 A | 2/1998  | Winterowd et al. |  |
| 5,238,534 A           | 8/1993           | Manning et al.           | 5,716,675 A | 2/1998  | Andersen et al.  |  |
| 5,260,017 A           | 11/1993          | Giles                    | 5,719,201 A | 2/1998  | Wilson           |  |
| 5,260,345 A           | 11/1993          | DesMarais et al.         | 5,720,851 A | 2/1998  | Reiner           |  |
| 5,268,224 A           | 12/1993          | DesMarais et al.         | 5,728,743 A | 3/1998  | Dyer et al.      |  |
| 5,300,565 A           | 4/1994           | Berg et al.              | 5,736,209 A | 4/1998  | Andersen et al.  |  |
| 5,308,565 A           | 5/1994           | Weber et al.             | 5,741,581 A | 4/1998  | DesMarais et al. |  |
| 5,318,554 A           | 6/1994           | Young et al.             | 5,744,506 A | 4/1998  | Goldman et al.   |  |
| 5,328,935 A           | 7/1994           | Van Phan et al.          | 5,744,509 A | 4/1998  | Wilson et al.    |  |
| 5,330,822 A           | 7/1994           | Berg et al.              | 5,753,308 A | 5/1998  | Andersen et al.  |  |
| 5,331,015 A           | 7/1994           | DesMarais et al.         | 5,753,359 A | 5/1998  | Dyer et al.      |  |
| 5,338,766 A           | 8/1994           | Phan et al.              | 5,763,499 A | 6/1998  | DesMarais        |  |
| 5,344,866 A           | 9/1994           | Hall                     | 5,770,634 A | 6/1998  | Dyer et al.      |  |
| 5,348,453 A           | 9/1994           | Baran et al.             | 5,776,388 A | 7/1998  | Andersen et al.  |  |

| (56) References Cited |         |                   |              |         |                     |
|-----------------------|---------|-------------------|--------------|---------|---------------------|
| U.S. PATENT DOCUMENTS |         |                   |              |         |                     |
| 5,783,126 A           | 7/1998  | Andersen et al.   | D437,119 S   | 2/2001  | Jahner et al.       |
| 5,795,921 A           | 8/1998  | Dyer et al.       | D437,120 S   | 2/2001  | Jahner et al.       |
| 5,800,416 A           | 9/1998  | Seger et al.      | D437,489 S   | 2/2001  | Jahner et al.       |
| 5,800,647 A           | 9/1998  | Andersen et al.   | D438,017 S   | 2/2001  | Reid                |
| 5,810,961 A           | 9/1998  | Andersen et al.   | 6,193,838 B1 | 2/2001  | Oriaran et al.      |
| 5,817,703 A           | 10/1998 | Blair et al.      | 6,200,404 B1 | 3/2001  | Andersen et al.     |
| 5,830,305 A           | 11/1998 | Andersen et al.   | 6,203,663 B1 | 3/2001  | Kamps et al.        |
| 5,843,055 A           | 12/1998 | Seger             | 6,207,244 B1 | 3/2001  | Hesch               |
| 5,843,544 A           | 12/1998 | Andersen et al.   | D440,051 S   | 4/2001  | Bredendick et al.   |
| 5,849,155 A           | 12/1998 | Gasland           | 6,214,907 B1 | 4/2001  | Tomka               |
| 5,849,805 A           | 12/1998 | Dyer              | 6,231,960 B1 | 5/2001  | Dyer et al.         |
| 5,851,634 A           | 12/1998 | Andersen et al.   | 6,231,970 B1 | 5/2001  | Andersen et al.     |
| 5,851,648 A           | 12/1998 | Stone et al.      | 6,235,816 B1 | 5/2001  | Lorcks et al.       |
| 5,853,402 A           | 12/1998 | Faulks et al.     | 6,238,518 B1 | 5/2001  | Rokman et al.       |
| 5,863,958 A           | 1/1999  | Dyer et al.       | D443,766 S   | 6/2001  | Bredendick et al.   |
| 5,868,724 A           | 2/1999  | Dierckes et al.   | 6,243,934 B1 | 6/2001  | Wadzinski           |
| 5,876,643 A           | 3/1999  | Biggs et al.      | 6,245,410 B1 | 6/2001  | Hähnle et al.       |
| 5,879,722 A           | 3/1999  | Andersen et al.   | 6,245,697 B1 | 6/2001  | Conrad et al.       |
| 5,882,479 A           | 3/1999  | Oriaran et al.    | 6,248,211 B1 | 6/2001  | Jennings et al.     |
| 5,899,893 A           | 5/1999  | Dyer et al.       | 6,251,207 B1 | 6/2001  | Schultz et al.      |
| 5,900,114 A           | 5/1999  | Brown et al.      | 6,258,203 B1 | 7/2001  | Rokman et al.       |
| 5,904,809 A           | 5/1999  | Rokman et al.     | 6,261,679 B1 | 7/2001  | Chen et al.         |
| 5,904,812 A           | 5/1999  | Salman et al.     | 6,274,077 B1 | 8/2001  | Hur et al.          |
| 5,908,533 A           | 6/1999  | Marinack et al.   | 6,280,570 B1 | 8/2001  | Harper et al.       |
| 5,916,503 A           | 6/1999  | Rettenbacher      | 6,287,417 B1 | 9/2001  | Bhat                |
| 5,916,928 A           | 6/1999  | Sessions et al.   | 6,287,422 B1 | 9/2001  | Harper et al.       |
| 5,919,411 A           | 7/1999  | Rezai et al.      | 6,296,736 B1 | 10/2001 | Hsu et al.          |
| 5,922,780 A           | 7/1999  | Dyer et al.       | 6,296,929 B1 | 10/2001 | Gentile et al.      |
| 5,925,299 A           | 7/1999  | Dierckes et al.   | 6,309,661 B1 | 10/2001 | Haynes et al.       |
| 5,928,741 A           | 7/1999  | Andersen et al.   | 6,328,850 B1 | 12/2001 | Phan et al.         |
| 5,948,829 A           | 9/1999  | Wallajapet et al. | D459,897 S   | 7/2002  | Bredendick et al.   |
| 5,958,186 A           | 9/1999  | Holm et al.       | 6,413,368 B1 | 7/2002  | Dwiggins et al.     |
| 5,976,235 A           | 11/1999 | Andersen et al.   | 6,419,790 B1 | 7/2002  | Leege et al.        |
| 5,985,434 A           | 11/1999 | Qin et al.        | 6,425,983 B1 | 7/2002  | Marinack et al.     |
| 6,001,218 A           | 12/1999 | Hsu et al.        | 6,432,272 B1 | 8/2002  | Hollenberg et al.   |
| 6,013,293 A           | 1/2000  | De Moor           | 6,436,234 B1 | 8/2002  | Chen et al.         |
| 6,013,589 A           | 1/2000  | DesMarais et al.  | 6,440,266 B1 | 8/2002  | George et al.       |
| 6,017,833 A           | 1/2000  | Reiner et al.     | 6,443,258 B1 | 9/2002  | Putt et al.         |
| 6,019,871 A           | 2/2000  | Rokman et al.     | 6,444,088 B2 | 9/2002  | Rokman et al.       |
| 6,022,615 A           | 2/2000  | Rettenbacher      | 6,447,640 B1 | 9/2002  | Watson et al.       |
| 6,027,610 A           | 2/2000  | Back et al.       | 6,451,166 B1 | 9/2002  | Marinack et al.     |
| 6,028,018 A           | 2/2000  | Amundson et al.   | 6,455,600 B1 | 9/2002  | Hähnle et al.       |
| 6,030,673 A           | 2/2000  | Andersen et al.   | 6,472,497 B2 | 10/2002 | Loercks et al.      |
| 6,037,282 A           | 3/2000  | Milding et al.    | 6,500,302 B2 | 12/2002 | Dwiggins et al.     |
| D423,232 S            | 4/2000  | Reid              | 6,503,372 B1 | 1/2003  | Rokman et al.       |
| 6,051,104 A           | 4/2000  | Oriaran et al.    | 6,518,479 B1 | 2/2003  | Graef et al.        |
| 6,054,022 A           | 4/2000  | Helwig et al.     | 6,525,240 B1 | 2/2003  | Graef et al.        |
| 6,074,527 A           | 6/2000  | Hsu et al.        | 6,527,913 B1 | 3/2003  | Johnson et al.      |
| 6,077,390 A           | 6/2000  | Salman et al.     | 6,531,078 B2 | 3/2003  | Laine et al.        |
| 6,077,590 A           | 6/2000  | Archer et al.     | 6,540,879 B2 | 4/2003  | Marinack et al.     |
| 6,083,211 A           | 7/2000  | DesMarais         | 6,544,386 B1 | 4/2003  | Krzysik et al.      |
| 6,083,586 A           | 7/2000  | Andersen et al.   | 6,548,132 B1 | 4/2003  | Clarke et al.       |
| 6,086,718 A           | 7/2000  | Carter et al.     | 6,562,193 B1 | 5/2003  | Elonen et al.       |
| 6,090,195 A           | 7/2000  | Andersen et al.   | 6,589,634 B2 | 7/2003  | Schultz et al.      |
| 6,093,359 A           | 7/2000  | Gauchel et al.    | 6,596,389 B1 | 7/2003  | Hallett et al.      |
| 6,096,809 A           | 8/2000  | Lorcks et al.     | 6,600,086 B1 | 7/2003  | Mace et al.         |
| 6,103,060 A           | 8/2000  | Munerelle et al.  | 6,603,054 B2 | 8/2003  | Chen et al.         |
| 6,103,063 A           | 8/2000  | Oriaran et al.    | 6,613,424 B1 | 9/2003  | Putt et al.         |
| D430,406 S            | 9/2000  | Ingalls           | 6,616,802 B1 | 9/2003  | Kinsley, Jr. et al. |
| D430,407 S            | 9/2000  | Ingalls           | 6,630,054 B1 | 10/2003 | Graef et al.        |
| D430,734 S            | 9/2000  | Bredendick et al. | 6,649,025 B2 | 11/2003 | Mills et al.        |
| 6,113,740 A           | 9/2000  | Oriaran et al.    | 6,657,101 B1 | 12/2003 | Malmgren et al.     |
| D431,371 S            | 10/2000 | Ingalls et al.    | 6,663,611 B2 | 12/2003 | Blaney et al.       |
| D431,372 S            | 10/2000 | Ingalls et al.    | 6,670,522 B1 | 12/2003 | Graef et al.        |
| 6,133,193 A           | 10/2000 | Kajikawa et al.   | 6,673,980 B1 | 1/2004  | Varona et al.       |
| 6,136,153 A           | 10/2000 | Rokman et al.     | 6,673,983 B1 | 1/2004  | Graef et al.        |
| 6,136,873 A           | 10/2000 | Hahnle et al.     | 6,682,215 B2 | 1/2004  | Kinsley, Jr. et al. |
| 6,153,053 A           | 11/2000 | Harper et al.     | 6,689,934 B2 | 2/2004  | Dodge, II et al.    |
| 6,160,028 A           | 12/2000 | Dyer              | 6,703,330 B1 | 3/2004  | Marsh               |
| 6,162,961 A           | 12/2000 | Tanner et al.     | 6,706,944 B2 | 3/2004  | Qin et al.          |
| 6,163,943 A           | 12/2000 | Johansson et al.  | 6,709,548 B2 | 3/2004  | Marinack et al.     |
| D436,738 S            | 1/2001  | Bredendick et al. | 6,709,550 B2 | 3/2004  | Holz et al.         |
| 6,168,857 B1          | 1/2001  | Andersen et al.   | 6,733,631 B2 | 5/2004  | Elonen et al.       |
| 6,174,152 B1          | 1/2001  | Rokman et al.     | 6,734,335 B1 | 5/2004  | Graef et al.        |
| 6,174,929 B1          | 1/2001  | Hnle et al.       | 6,746,570 B2 | 6/2004  | Burazin et al.      |

| (56)                  | References Cited |                       |              |         |                     |  |
|-----------------------|------------------|-----------------------|--------------|---------|---------------------|--|
| U.S. PATENT DOCUMENTS |                  |                       |              |         |                     |  |
| 6,749,719 B2          | 6/2004           | Burazin et al.        | 7,435,266 B2 | 10/2008 | Sun et al.          |  |
| 6,750,262 B1          | 6/2004           | Hähnle et al.         | 7,435,313 B2 | 10/2008 | Boatman et al.      |  |
| 6,752,907 B2          | 6/2004           | Edwards et al.        | 7,435,316 B2 | 10/2008 | Boatman et al.      |  |
| 6,780,356 B1          | 8/2004           | Putt et al.           | 7,494,563 B2 | 2/2009  | Edwards et al.      |  |
| 6,787,000 B2          | 9/2004           | Burazin et al.        | 7,497,923 B2 | 3/2009  | Ward et al.         |  |
| 6,790,314 B2          | 9/2004           | Burazin et al.        | 7,497,925 B2 | 3/2009  | Hermans et al.      |  |
| 6,797,114 B2          | 9/2004           | Hu                    | 7,497,926 B2 | 3/2009  | Hermans et al.      |  |
| 6,808,790 B2          | 10/2004          | Chen et al.           | 7,503,998 B2 | 3/2009  | Hermans et al.      |  |
| 6,821,385 B2          | 11/2004          | Burazin et al.        | 7,524,399 B2 | 4/2009  | Murray et al.       |  |
| 6,821,387 B2          | 11/2004          | Hu                    | 7,524,404 B2 | 4/2009  | Boatman et al.      |  |
| 6,821,388 B2          | 11/2004          | Marsh                 | 7,585,388 B2 | 9/2009  | Yeh et al.          |  |
| 6,824,650 B2          | 11/2004          | Lindsay et al.        | 7,585,389 B2 | 9/2009  | Yeh et al.          |  |
| 6,830,656 B2          | 12/2004          | Kinsley, Jr.          | 7,597,777 B2 | 10/2009 | Wilke, II           |  |
| 6,837,956 B2          | 1/2005           | Cowell et al.         | 7,601,374 B2 | 10/2009 | Clarke              |  |
| 6,837,972 B2          | 1/2005           | Marsh                 | 7,629,043 B2 | 12/2009 | Lindsay et al.      |  |
| 6,861,380 B2          | 3/2005           | Garnier et al.        | 7,645,359 B2 | 1/2010  | Lorenz et al.       |  |
| 6,861,477 B2          | 3/2005           | Wang et al.           | 7,662,257 B2 | 2/2010  | Edwards et al.      |  |
| 6,867,346 B1          | 3/2005           | Dopps et al.          | 7,670,457 B2 | 3/2010  | Murray et al.       |  |
| 6,875,315 B2          | 4/2005           | Bakken et al.         | 7,678,229 B2 | 3/2010  | Wilke, II           |  |
| 6,878,238 B2          | 4/2005           | Bakken et al.         | 7,678,231 B2 | 3/2010  | Dyer et al.         |  |
| 6,887,348 B2          | 5/2005           | Hermans et al.        | 7,682,697 B2 | 3/2010  | Raghavendran et al. |  |
| 6,887,350 B2          | 5/2005           | Garnier et al.        | 7,691,228 B2 | 4/2010  | Edwards et al.      |  |
| 6,893,535 B2          | 5/2005           | Hermans et al.        | 7,699,959 B2 | 4/2010  | Ward et al.         |  |
| 6,921,459 B2          | 7/2005           | Kinsley, Jr. et al.   | 7,744,576 B2 | 6/2010  | Busam et al.        |  |
| 6,924,030 B2 *        | 8/2005           | Kamada .....          | 7,750,203 B2 | 7/2010  | Becker et al.       |  |
|                       |                  | D01D 5/253            | 7,775,958 B2 | 8/2010  | Mukai et al.        |  |
|                       |                  | 264/185               | 7,785,696 B2 | 8/2010  | Boatman et al.      |  |
|                       |                  |                       | 7,794,565 B2 | 9/2010  | Shannon et al.      |  |
|                       |                  |                       | 7,799,161 B2 | 9/2010  | Schuh et al.        |  |
|                       |                  |                       | 7,799,968 B2 | 9/2010  | Chen et al.         |  |
| 6,939,914 B2          | 9/2005           | Qin et al.            | 7,820,008 B2 | 10/2010 | Edwards et al.      |  |
| 6,946,058 B2          | 9/2005           | Hu                    | 7,828,932 B2 | 11/2010 | Hermans et al.      |  |
| 6,951,598 B2          | 10/2005          | Flugge et al.         | 7,846,296 B2 | 12/2010 | Luu et al.          |  |
| 6,956,009 B2          | 10/2005          | Wang et al.           | 7,850,823 B2 | 12/2010 | Chou et al.         |  |
| 6,962,645 B2          | 11/2005          | Graef et al.          | 7,851,057 B2 | 12/2010 | Englert et al.      |  |
| 6,964,725 B2          | 11/2005          | Shannon et al.        | 7,851,667 B2 | 12/2010 | Becker et al.       |  |
| 6,969,781 B2          | 11/2005          | Graef et al.          | 7,857,941 B2 | 12/2010 | Ruthven et al.      |  |
| 6,983,821 B2          | 1/2006           | Putt et al.           | 7,862,686 B2 | 1/2011  | Ward et al.         |  |
| D517,816 S            | 3/2006           | Dwiggins et al.       | 7,887,676 B2 | 2/2011  | Boatman et al.      |  |
| 7,029,756 B2          | 4/2006           | Moline et al.         | 7,918,951 B2 | 4/2011  | Lorenz et al.       |  |
| D519,739 S            | 5/2006           | Schuh et al.          | 7,918,964 B2 | 4/2011  | Edwards et al.      |  |
| 7,041,196 B2          | 5/2006           | Lorenz et al.         | 7,918,972 B2 | 4/2011  | Boatman et al.      |  |
| 7,045,026 B2          | 5/2006           | Lorenz et al.         | 7,927,456 B2 | 4/2011  | Murray et al.       |  |
| 7,052,580 B2          | 5/2006           | Trokhan et al.        | 7,972,476 B2 | 7/2011  | Scherb et al.       |  |
| 7,066,006 B2          | 6/2006           | Minerath, III et al.  | 7,994,079 B2 | 8/2011  | Chen et al.         |  |
| 7,067,038 B2          | 6/2006           | Trokhan et al.        | 8,007,640 B2 | 8/2011  | Boatman et al.      |  |
| 7,081,559 B2          | 7/2006           | Fujikawa et al.       | 8,017,827 B2 | 9/2011  | Hundorf et al.      |  |
| 7,125,470 B2          | 10/2006          | Graef et al.          | 8,056,733 B2 | 11/2011 | Koslow              |  |
| 7,141,142 B2          | 11/2006          | Burazin et al.        | 8,083,893 B2 | 12/2011 | Boatman et al.      |  |
| 7,155,991 B2          | 1/2007           | Minerath, III et al.  | 8,092,848 B2 | 1/2012  | Clarke              |  |
| 7,156,954 B2          | 1/2007           | Farrington, Jr et al. | 8,102,275 B2 | 1/2012  | McGuire et al.      |  |
| 7,160,418 B2          | 1/2007           | Edwards et al.        | 8,110,232 B2 | 2/2012  | Clarke              |  |
| 7,166,190 B2          | 1/2007           | Graef et al.          | 8,123,905 B2 | 2/2012  | Luu et al.          |  |
| 7,169,451 B2          | 1/2007           | Clarke et al.         | 8,142,612 B2 | 3/2012  | Murray et al.       |  |
| 7,214,293 B2          | 5/2007           | Trokhan et al.        | 8,142,617 B2 | 3/2012  | Ruthven et al.      |  |
| 7,220,821 B2          | 5/2007           | Hähnle et al.         | 8,143,472 B1 | 3/2012  | Bragd et al.        |  |
| 7,229,528 B2          | 6/2007           | Vinson et al.         | 8,152,957 B2 | 4/2012  | Edwards et al.      |  |
| 7,235,708 B2          | 6/2007           | Guidotti et al.       | 8,152,958 B2 | 4/2012  | Super et al.        |  |
| D551,406 S            | 9/2007           | Caruso et al.         | 8,158,689 B2 | 4/2012  | Baker et al.        |  |
| 7,285,183 B2          | 10/2007          | Kajander et al.       | 8,178,025 B2 | 5/2012  | Awofeso et al.      |  |
| 7,287,650 B2          | 10/2007          | Koslow                | 8,187,240 B2 | 5/2012  | Busam et al.        |  |
| 7,291,382 B2          | 11/2007          | Krueger et al.        | 8,187,427 B2 | 5/2012  | Schuh et al.        |  |
| 7,294,238 B2          | 11/2007          | Bakken et al.         | 8,211,078 B2 | 7/2012  | Noel                |  |
| 7,300,547 B2          | 11/2007          | Luu et al.            | 8,226,797 B2 | 7/2012  | Murray et al.       |  |
| 7,311,800 B2          | 12/2007          | Russell et al.        | 8,257,552 B2 | 9/2012  | Edwards et al.      |  |
| 7,314,663 B2          | 1/2008           | Stelljes, Jr. et al.  | 8,293,072 B2 | 10/2012 | Super et al.        |  |
| 7,314,664 B2          | 1/2008           | Stelljes, Jr. et al.  | 8,319,005 B2 | 11/2012 | Becker et al.       |  |
| 7,314,665 B2          | 1/2008           | Stelljes, Jr. et al.  | 8,324,446 B2 | 12/2012 | Wang et al.         |  |
| 7,322,970 B2          | 1/2008           | Schmidt et al.        | 8,328,985 B2 | 12/2012 | Edwards et al.      |  |
| 7,354,502 B2          | 4/2008           | Polat et al.          | 8,361,278 B2 | 1/2013  | Fike et al.         |  |
| 7,364,015 B2          | 4/2008           | Englert et al.        | 8,378,000 B2 | 2/2013  | Hintz et al.        |  |
| 7,374,638 B2          | 5/2008           | Horenziak et al.      | 8,388,803 B2 | 3/2013  | Super et al.        |  |
| 7,390,378 B2          | 6/2008           | Carels et al.         | 8,388,804 B2 | 3/2013  | Super et al.        |  |
| 7,396,436 B2          | 7/2008           | Trokhan et al.        | 8,394,236 B2 | 3/2013  | Edwards et al.      |  |
| 7,407,560 B2          | 8/2008           | Hilbig et al.         | 8,398,818 B2 | 3/2013  | Edwards et al.      |  |
| 7,413,629 B2          | 8/2008           | Fisher et al.         | 8,398,820 B2 | 3/2013  | Edwards et al.      |  |
| 7,416,636 B2 *        | 8/2008           | Blomqvist .....       | 8,425,721 B2 | 4/2013  | Tynkkynen et al.    |  |
|                       |                  | D21F 11/002           | 8,435,381 B2 | 5/2013  | Murray et al.       |  |
|                       |                  | 162/101               | 8,461,412 B2 | 6/2013  | Febo et al.         |  |
| 7,416,637 B2          | 8/2008           | Murray et al.         |              |         |                     |  |

| (56)                  | References Cited |                      |
|-----------------------|------------------|----------------------|
| U.S. PATENT DOCUMENTS |                  |                      |
| 8,496,637 B2          | 7/2013           | Hundorf et al.       |
| 8,512,516 B2          | 8/2013           | Murray et al.        |
| 8,524,040 B2          | 9/2013           | Edwards et al.       |
| 8,540,846 B2          | 9/2013           | Miller et al.        |
| 8,545,676 B2          | 10/2013          | Super et al.         |
| 8,552,252 B2          | 10/2013          | Hundorf et al.       |
| 8,562,786 B2          | 10/2013          | Murray et al.        |
| 8,568,559 B2          | 10/2013          | Murray et al.        |
| 8,568,560 B2          | 10/2013          | Murray et al.        |
| 8,603,296 B2          | 12/2013          | Edwards et al.       |
| 8,632,658 B2          | 1/2014           | Miller et al.        |
| 8,636,874 B2          | 1/2014           | Super et al.         |
| 8,647,105 B2          | 2/2014           | Awofeso et al.       |
| 8,652,300 B2          | 2/2014           | Super et al.         |
| 8,662,344 B2          | 3/2014           | Gispert              |
| 8,673,115 B2          | 3/2014           | Edwards et al.       |
| 8,674,170 B2          | 3/2014           | Busam et al.         |
| 8,702,668 B2          | 4/2014           | Noel                 |
| 8,741,105 B2          | 6/2014           | Beaupre et al.       |
| 8,766,031 B2          | 7/2014           | Becker et al.        |
| 8,778,138 B2          | 7/2014           | Super et al.         |
| 8,791,318 B2          | 7/2014           | Becker et al.        |
| 8,815,056 B2          | 8/2014           | Araki et al.         |
| 8,829,263 B2          | 9/2014           | Haggstrom et al.     |
| 8,841,506 B2          | 9/2014           | Febo et al.          |
| 8,852,397 B2          | 10/2014          | Super et al.         |
| 8,864,944 B2          | 10/2014          | Miller et al.        |
| 8,864,945 B2          | 10/2014          | Miller et al.        |
| 8,911,592 B2          | 12/2014          | Edwards et al.       |
| 8,968,516 B2          | 3/2015           | Super et al.         |
| 8,979,815 B2          | 3/2015           | Roe et al.           |
| 8,980,052 B2          | 3/2015           | Super et al.         |
| 9,017,517 B2          | 4/2015           | Super et al.         |
| 9,044,359 B2          | 6/2015           | Wciorka et al.       |
| 9,051,691 B2          | 6/2015           | Miller et al.        |
| 9,057,158 B2          | 6/2015           | Miller et al.        |
| 9,138,360 B1          | 9/2015           | Febo et al.          |
| 9,144,524 B2          | 9/2015           | Febo et al.          |
| 9,216,116 B2          | 12/2015          | Roe et al.           |
| 9,216,118 B2          | 12/2015          | Roe et al.           |
| 9,228,048 B2          | 1/2016           | Wibaux et al.        |
| 9,241,845 B2          | 1/2016           | Hundorf et al.       |
| 9,243,367 B2          | 1/2016           | Rekoske et al.       |
| 9,267,240 B2          | 2/2016           | Lee et al.           |
| 9,279,219 B2          | 3/2016           | Edwards et al.       |
| 9,309,627 B2          | 4/2016           | Miller et al.        |
| 9,326,896 B2          | 5/2016           | Schafer et al.       |
| 9,333,120 B2          | 5/2016           | Lavon et al.         |
| 9,334,610 B2          | 5/2016           | Kinnunen et al.      |
| 9,340,363 B2          | 5/2016           | Jackels et al.       |
| 9,365,977 B2          | 6/2016           | Beaupre et al.       |
| 9,371,614 B2          | 6/2016           | Schuh et al.         |
| 9,371,615 B2          | 6/2016           | Super et al.         |
| 9,375,358 B2          | 6/2016           | Ehmsperger et al.    |
| 9,382,665 B2          | 7/2016           | Miller et al.        |
| 9,388,534 B2          | 7/2016           | Super et al.         |
| 9,447,543 B2          | 9/2016           | Matula               |
| 9,468,566 B2          | 10/2016          | Rosati et al.        |
| 9,476,162 B2          | 10/2016          | Lee et al.           |
| 9,492,328 B2          | 11/2016          | Jackels et al.       |
| 9,493,911 B2          | 11/2016          | Miller et al.        |
| 9,532,910 B2          | 1/2017           | Rosati et al.        |
| 9,572,728 B2          | 2/2017           | Ashton et al.        |
| 9,579,238 B2          | 2/2017           | Noel                 |
| 9,603,755 B2          | 3/2017           | Tanaka               |
| 9,649,232 B2          | 5/2017           | Hippe et al.         |
| 9,649,830 B2          | 5/2017           | Rasch                |
| 9,657,443 B2          | 5/2017           | Rekoske et al.       |
| 9,662,246 B2          | 5/2017           | Collinson et al.     |
| 9,668,926 B2          | 6/2017           | Jackels et al.       |
| 9,708,774 B2          | 7/2017           | Lee et al.           |
| 9,713,556 B2          | 7/2017           | Arizti et al.        |
| 9,713,557 B2          | 7/2017           | Arizti et al.        |
| 9,739,015 B2          | 8/2017           | Miller et al.        |
| 9,744,755 B2          | 8/2017           | Thompson, Jr. et al. |
|                       |                  | 9,752,280 B2         |
|                       |                  | 9,763,835 B2         |
|                       |                  | 9,789,009 B2         |
|                       |                  | 9,789,011 B2         |
|                       |                  | 9,808,554 B2         |
|                       |                  | 9,822,487 B2         |
|                       |                  | 9,877,872 B2         |
|                       |                  | 9,879,382 B2         |
|                       |                  | 9,950,309 B2         |
|                       |                  | 9,963,568 B2         |
|                       |                  | 9,974,697 B2         |
|                       |                  | 9,974,699 B2         |
|                       |                  | 9,987,176 B2         |
|                       |                  | 9,988,763 B2         |
|                       |                  | 9,994,712 B2         |
|                       |                  | 9,995,005 B2         |
|                       |                  | 10,004,647 B2        |
|                       |                  | 10,022,280 B2        |
|                       |                  | 10,034,800 B2        |
|                       |                  | 10,039,673 B2        |
|                       |                  | 10,039,676 B2        |
|                       |                  | 10,052,242 B2        |
|                       |                  | 10,065,175 B2        |
|                       |                  | 10,071,002 B2        |
|                       |                  | 10,076,449 B2        |
|                       |                  | 10,099,425 B2        |
|                       |                  | 10,130,519 B2        |
|                       |                  | 10,130,525 B2        |
|                       |                  | 10,130,527 B2        |
|                       |                  | 10,137,039 B2        |
|                       |                  | 10,138,600 B2        |
|                       |                  | 10,149,788 B2        |
|                       |                  | 10,190,263 B2        |
|                       |                  | 10,196,780 B2        |
|                       |                  | 10,201,644 B2        |
|                       |                  | 10,208,426 B2        |
|                       |                  | 10,221,350 B2        |
|                       |                  | 10,231,874 B2        |
|                       |                  | 10,245,188 B2        |
|                       |                  | 10,247,195 B2        |
|                       |                  | 10,253,434 B2 *      |
|                       |                  | 10,259,151 B2        |
|                       |                  | 10,273,635 B2        |
|                       |                  | 10,292,875 B2        |
|                       |                  | 10,301,775 B2        |
|                       |                  | 10,301,779 B2        |
|                       |                  | 10,322,040 B2        |
|                       |                  | 10,335,324 B2        |
|                       |                  | 10,619,303 B2        |
|                       |                  | 11,015,292 B2        |
|                       |                  | 11,136,700 B2        |
|                       |                  | 2001/0013389 A1      |
|                       |                  | 2002/0007169 A1      |
|                       |                  | 2002/0013560 A1      |
|                       |                  | 2002/0055310 A1      |
|                       |                  | 2002/0088581 A1      |
|                       |                  | 2002/0092634 A1      |
|                       |                  | 2002/0132121 A1      |
|                       |                  | 2003/0106656 A1      |
|                       |                  | 2003/0134094 A1      |
|                       |                  | 2003/0139715 A1      |
|                       |                  | 2003/0167045 A1      |
|                       |                  | 2003/0171727 A1      |
|                       |                  | 2003/0220039 A1      |
|                       |                  | 2004/0045685 A1      |
|                       |                  | 2004/0063367 A1      |
|                       |                  | 2004/0065420 A1      |
|                       |                  | 2004/0084162 A1      |
|                       |                  | 2004/0084164 A1      |
|                       |                  | 2004/0096642 A1      |
|                       |                  | 2004/0110017 A1      |
|                       |                  | 2004/0111817 A1      |
|                       |                  | 2004/0112783 A1      |
|                       |                  | 2004/0115419 A1      |
|                       |                  | 2004/0115451 A1      |
|                       |                  | 2004/0118530 A1      |
|                       |                  | 2004/0121680 A1      |
|                       |                  | 2004/0127873 A1      |
|                       |                  | 2004/0142620 A1      |
|                       |                  | 2005/0001389 A1      |
|                       |                  | 2005/0007169 A1      |
|                       |                  | 2005/0013560 A1      |
|                       |                  | 2005/0055310 A1      |
|                       |                  | 2005/0088581 A1      |
|                       |                  | 2005/0092634 A1      |
|                       |                  | 2005/0132121 A1      |
|                       |                  | 2006/0106656 A1      |
|                       |                  | 2006/0134094 A1      |
|                       |                  | 2006/0139715 A1      |
|                       |                  | 2006/0167045 A1      |
|                       |                  | 2006/0171727 A1      |
|                       |                  | 2006/0220039 A1      |
|                       |                  | 2007/0045685 A1      |
|                       |                  | 2007/0063367 A1      |
|                       |                  | 2007/0065420 A1      |
|                       |                  | 2007/0084162 A1      |
|                       |                  | 2007/0084164 A1      |
|                       |                  | 2007/0096642 A1      |
|                       |                  | 2007/0110017 A1      |
|                       |                  | 2007/0111817 A1      |
|                       |                  | 2007/0112783 A1      |
|                       |                  | 2007/0115419 A1      |
|                       |                  | 2007/0115451 A1      |
|                       |                  | 2007/0118530 A1      |
|                       |                  | 2007/0121680 A1      |
|                       |                  | 2007/0127873 A1      |
|                       |                  | 2007/0142620 A1      |
|                       |                  | 2008/0001389 A1      |
|                       |                  | 2008/0007169 A1      |
|                       |                  | 2008/0013560 A1      |
|                       |                  | 2008/0055310 A1      |
|                       |                  | 2008/0088581 A1      |
|                       |                  | 2008/0092634 A1      |
|                       |                  | 2008/0132121 A1      |
|                       |                  | 2008/0106656 A1      |
|                       |                  | 2008/0134094 A1      |
|                       |                  | 2008/0139715 A1      |
|                       |                  | 2008/0167045 A1      |
|                       |                  | 2008/0171727 A1      |
|                       |                  | 2008/0220039 A1      |
|                       |                  | 2009/0045685 A1      |
|                       |                  | 2009/0063367 A1      |
|                       |                  | 2009/0065420 A1      |
|                       |                  | 2009/0084162 A1      |
|                       |                  | 2009/0084164 A1      |
|                       |                  | 2009/0096642 A1      |
|                       |                  | 2009/0110017 A1      |
|                       |                  | 2009/0111817 A1      |
|                       |                  | 2009/0112783 A1      |
|                       |                  | 2009/0115419 A1      |
|                       |                  | 2009/0115451 A1      |
|                       |                  | 2009/0118530 A1      |
|                       |                  | 2009/0121680 A1      |
|                       |                  | 2009/0127873 A1      |
|                       |                  | 2009/0142620 A1      |
|                       |                  | 2010/0001389 A1      |
|                       |                  | 2010/0007169 A1      |
|                       |                  | 2010/0013560 A1      |
|                       |                  | 2010/0055310 A1      |
|                       |                  | 2010/0088581 A1      |
|                       |                  | 2010/0092634 A1      |
|                       |                  | 2010/0132121 A1      |
|                       |                  | 2010/0106656 A1      |
|                       |                  | 2010/0134094 A1      |
|                       |                  | 2010/0139715 A1      |
|                       |                  | 2010/0167045 A1      |
|                       |                  | 2010/0171727 A1      |
|                       |                  | 2010/0220039 A1      |
|                       |                  | 2011/0045685 A1      |
|                       |                  | 2011/0063367 A1      |
|                       |                  | 2011/0065420 A1      |
|                       |                  | 2011/0084162 A1      |
|                       |                  | 2011/0084164 A1      |
|                       |                  | 2011/0096642 A1      |
|                       |                  | 2011/0110017 A1      |
|                       |                  | 2011/0111817 A1      |
|                       |                  | 2011/0112783 A1      |
|                       |                  | 2011/0115419 A1      |
|                       |                  | 2011/0115451 A1      |
|                       |                  | 2011/0118530 A1      |
|                       |                  | 2011/0121680 A1      |
|                       |                  | 2011/0127873 A1      |
|                       |                  | 2011/0142620 A1      |
|                       |                  | 2012/0001389 A1      |
|                       |                  | 2012/0007169 A1      |
|                       |                  | 2012/0013560 A1      |
|                       |                  | 2012/0055310 A1      |
|                       |                  | 2012/0088581 A1      |
|                       |                  | 2012/0092634 A1      |
|                       |                  | 2012/0132121 A1      |
|                       |                  | 2012/0106656 A1      |
|                       |                  | 2012/0134094 A1      |
|                       |                  | 2012/0139715 A1      |
|                       |                  | 2012/0167045 A1      |
|                       |                  | 2012/0171727 A1      |
|                       |                  | 2012/0220039 A1      |
|                       |                  | 2013/0045685 A1      |
|                       |                  | 2013/0063367 A1      |
|                       |                  | 2013/0065420 A1      |
|                       |                  | 2013/0084162 A1      |
|                       |                  | 2013/0084164 A1      |
|                       |                  | 2013/0096642 A1      |
|                       |                  | 2013/0110017 A1      |
|                       |                  | 2013/0111817 A1      |
|                       |                  | 2013/0112783 A1      |
|                       |                  | 2013/0115419 A1      |
|                       |                  | 2013/0115451 A1      |
|                       |                  | 2013/0118530 A1      |
|                       |                  | 2013/0121680 A1      |
|                       |                  | 2013/0127873 A1      |
|                       |                  | 2013/0142620 A1      |
|                       |                  | 2014/0001389 A1      |
|                       |                  | 2014/0007169 A1      |
|                       |                  | 2014/0013560 A1      |
|                       |                  | 2014/0055310 A1      |
|                       |                  | 2014/0088581 A1      |
|                       |                  | 2014/0092634 A1      |
|                       |                  | 2014/0132121 A1      |
|                       |                  | 2014/0106656 A1      |
|                       |                  | 2014/0134094 A1      |
|                       |                  | 2014/0139715 A1      |
|                       |                  | 2014/0167045 A1      |
|                       |                  | 2014/0171727 A1      |
|                       |                  | 2014/0220039 A1      |
|                       |                  | 2015/0045685 A1      |
|                       |                  | 2015/0063367 A1      |
|                       |                  | 2015/0065420 A1      |
|                       |                  | 2015/0084162 A1      |
|                       |                  | 2015/0084164 A1      |
|                       |                  | 2015/0096642 A1      |
|                       |                  | 2015/0110017 A1      |
|                       |                  | 2015/0111817 A1      |
|                       |                  | 2015/0112783 A1      |
|                       |                  | 2015/0115419 A1      |
|                       |                  | 2015/0115451 A1      |
|                       |                  | 2015/0118530 A1      |
|                       |                  | 2015/0121680 A1      |
|                       |                  | 2015/0127873 A1      |
|                       |                  | 2015/0142620 A1      |
|                       |                  | 2016/0001389 A1      |
|                       |                  | 2016/0007169 A1      |
|                       |                  | 2016/0013560 A1      |
|                       |                  | 2016/0055310 A1      |
|                       |                  | 2016/0088581 A1      |
|                       |                  | 2016/0092634 A1      |
|                       |                  | 2016/0132121 A1      |
|                       |                  | 2016/0106656 A1      |
|                       |                  | 2016/0134094 A1      |
|                       |                  | 2016/0139715 A1      |
|                       |                  | 2016/0167045 A1      |
|                       |                  | 2016/0171727 A1      |
|                       |                  | 2016/0220039 A1      |
|                       |                  | 2017/0045685 A1      |
|                       |                  | 2017/0063367 A1      |
|                       |                  | 2017/0065420 A1      |
|                       |                  | 2017/0084162 A1      |
|                       |                  | 2017/0084164 A1      |
|                       |                  | 2017/0096642 A1      |
|                       |                  | 2017/0110017 A1      |
|                       |                  | 2017/0111817 A1      |
|                       |                  | 2017/0112783 A1      |
|                       |                  | 2017/0115419 A1      |
|                       |                  | 2017/0115451 A1      |
|                       |                  | 2017/0118530 A1      |
|                       |                  | 2017/0121680 A1      |
|                       |                  | 2017/0127873 A1      |
|                       |                  | 2017/0142620 A1      |
|                       |                  | 2018/0001389 A1      |
|                       |                  | 2018/0007169 A1      |
|                       |                  | 2018/0013560 A1      |
|                       |                  | 2018/0055310 A1      |
|                       |                  | 2018/0088581 A1      |
|                       |                  | 2018/0092634 A1      |
|                       |                  | 2018/0132121 A1      |
|                       |                  | 2018/0106656 A1      |
|                       |                  | 2018/0134094 A1      |
|                       |                  | 2018/0139715 A1      |
|                       |                  | 2018/0167045 A1      |
|                       |                  | 2018/0171727 A1      |
|                       |                  | 2018/0220039 A1      |
|                       |                  | 2019/0045685 A1      |
|                       |                  | 2019/0063367 A1      |
|                       |                  |                      |

# US 11,255,051 B2

Page 6

| (56) References Cited |         |                   |                  |                                          |
|-----------------------|---------|-------------------|------------------|------------------------------------------|
| U.S. PATENT DOCUMENTS |         |                   |                  |                                          |
| 2004/0157524 A1       | 8/2004  | Polat et al.      | 2017/0335521 A1  | 11/2017 Lee                              |
| 2004/0254551 A1       | 12/2004 | Carnes et al.     | 2017/0335522 A1  | 11/2017 Heiskanen et al.                 |
| 2004/0256066 A1       | 12/2004 | Lindsay et al.    | 2017/0362775 A1  | 12/2017 Juvonen et al.                   |
| 2005/0034826 A1       | 2/2005  | Hu                | 2018/0119353 A1  | 5/2018 Tolfsson et al.                   |
| 2005/0039870 A1*      | 2/2005  | Blomqvist .....   | D21F 11/002      | 2018/0140529 A1* 5/2018 Miller, IV ..... |
|                       |         |                   | 162/101          | A61K 8/66                                |
| 2005/0060933 A1       | 3/2005  | Henson            | 2018/0162107 A1* | 6/2018 Xu .....                          |
| 2005/0090789 A1       | 4/2005  | Graef et al.      | 2018/0327973 A1  | 11/2018 Siitonem et al.                  |
| 2005/0095980 A1       | 5/2005  | Chang             | 2018/0355527 A1  | 12/2018 Strandqvist et al.               |
| 2005/0106223 A1       | 5/2005  | Kelly             | 2019/0161915 A1  | 5/2019 Swails et al.                     |
| 2005/0124709 A1       | 6/2005  | Krueger et al.    | 2020/0190739 A1* | 6/2020 Qin .....                         |
| 2005/0136772 A1       | 6/2005  | Chen et al.       | 2020/0370246 A1* | 11/2020 Calewarts .....                  |
| 2005/0142348 A1       | 6/2005  | Kajander et al.   | D21H 15/10       | D04H 1/5412                              |
| 2005/0152954 A1       | 7/2005  | Farrell et al.    |                  |                                          |
| 2005/0230069 A1       | 10/2005 | Hilbig et al.     |                  |                                          |
| 2005/0244627 A1       | 11/2005 | Travelute et al.  |                  |                                          |
| 2005/0247397 A1       | 11/2005 | Kraus et al.      |                  |                                          |
| 2005/0247416 A1       | 11/2005 | Forry et al.      |                  |                                          |
| 2005/0267226 A1       | 12/2005 | Wehr et al.       |                  |                                          |
| 2006/0005916 A1       | 1/2006  | Stelljes et al.   |                  |                                          |
| 2006/0011315 A1       | 1/2006  | Kinsley et al.    |                  |                                          |
| 2006/0030632 A1       | 2/2006  | Krueger et al.    |                  |                                          |
| 2006/0081348 A1       | 4/2006  | Graef et al.      |                  |                                          |
| 2006/0135026 A1       | 6/2006  | Arendt et al.     |                  |                                          |
| 2006/0141880 A1       | 6/2006  | Bascom et al.     |                  |                                          |
| 2006/0142719 A1       | 6/2006  | Vogt et al.       |                  |                                          |
| 2006/0191357 A1       | 8/2006  | Minerath et al.   |                  |                                          |
| 2006/0266485 A1       | 11/2006 | Knox et al.       |                  |                                          |
| 2006/0266487 A1       | 11/2006 | Scherb et al.     |                  |                                          |
| 2007/0148433 A1       | 6/2007  | Mallory et al.    |                  |                                          |
| 2007/0179210 A1       | 8/2007  | Swaniker          |                  |                                          |
| 2007/0218485 A1       | 9/2007  | Davis et al.      |                  |                                          |
| 2007/0269644 A1       | 11/2007 | Harper et al.     |                  |                                          |
| 2008/0052859 A1       | 3/2008  | Orlandi           |                  |                                          |
| 2008/0179775 A1       | 7/2008  | Palm et al.       |                  |                                          |
| 2008/0312617 A1       | 12/2008 | Hundorf et al.    |                  |                                          |
| 2008/0312618 A1       | 12/2008 | Hundorf et al.    |                  |                                          |
| 2008/0312619 A1       | 12/2008 | Ashton et al.     |                  |                                          |
| 2008/0312620 A1       | 12/2008 | Ashton et al.     |                  |                                          |
| 2008/0312621 A1       | 12/2008 | Hundorf et al.    |                  |                                          |
| 2008/0312622 A1       | 12/2008 | Hundorf et al.    |                  |                                          |
| 2008/0312625 A1       | 12/2008 | Hundorf et al.    |                  |                                          |
| 2008/0312628 A1       | 12/2008 | Hundorf et al.    |                  |                                          |
| 2009/0000753 A1       | 1/2009  | Vestola et al.    |                  |                                          |
| 2009/0001635 A1       | 1/2009  | Newson et al.     |                  |                                          |
| 2009/0008275 A1       | 1/2009  | Ferrari et al.    |                  |                                          |
| 2009/0117365 A1       | 5/2009  | Mallory et al.    |                  |                                          |
| 2009/0131898 A1       | 5/2009  | Malmgren et al.   |                  |                                          |
| 2009/0205794 A1       | 8/2009  | Scherb et al.     |                  |                                          |
| 2009/0270005 A1       | 10/2009 | Takahashi et al.  |                  |                                          |
| 2010/0006498 A1*      | 1/2010  | Duello .....      | B32B 5/26        | DE 2041406 A1 4/1971                     |
|                       |         |                   | 210/508          | DE 2438587 A1 3/1975                     |
|                       |         |                   |                  | DE 2902255 A1 7/1980                     |
| 2010/0075858 A1       | 3/2010  | Davis et al.      |                  | DE 3307736 A1 9/1984                     |
| 2010/0132144 A1       | 6/2010  | Rautray           |                  | DE 3420195 C2 6/1987                     |
| 2010/0136294 A1       | 6/2010  | Manifold et al.   |                  | DE 4207233 A1 11/1993                    |
| 2010/0251611 A1       | 10/2010 | Henson            | EP 0101319 A3    | 3/1984                                   |
| 2010/0273716 A1       | 10/2010 | Harris            | EP 3049944 B1    | 11/1984                                  |
| 2010/0327484 A1       | 12/2010 | Schuh et al.      | EP 0264676 A1    | 4/1988                                   |
| 2011/0045261 A1       | 2/2011  | Sellars           | EP 0136329 A4    | 1/1989                                   |
| 2012/0121674 A1       | 5/2012  | Pedoja            | EP 0158938 B1    | 12/1989                                  |
| 2012/0177888 A1       | 7/2012  | Escafere et al.   | EP 0296242 A4    | 7/1991                                   |
| 2013/0268062 A1       | 10/2013 | Puckett et al.    | EP 0443082 A1    | 8/1991                                   |
| 2014/0102650 A1       | 4/2014  | Qin et al.        | EP 0242361 B1    | 9/1991                                   |
| 2014/0189970 A1       | 7/2014  | Fingal et al.     | EP 0512819 A1    | 11/1992                                  |
| 2014/0231037 A1       | 8/2014  | Beaupre et al.    | EP 0150777 B2    | 11/1994                                  |
| 2014/0324007 A1       | 10/2014 | Hundorf et al.    | EP 0481745 B1    | 7/1996                                   |
| 2015/0080823 A1       | 3/2015  | Thompson et al.   | EP 0537005 B1    | 7/1997                                   |
| 2015/0144829 A1       | 5/2015  | Grünbauer         | EP 0671504 B1    | 8/1997                                   |
| 2015/0284911 A1       | 10/2015 | Juvonen et al.    | EP 0742858 B1    | 6/1999                                   |
| 2015/0330029 A1*      | 11/2015 | Ramaratnam .....  | B32B 3/30        | EP 0951603 B1 8/2002                     |
|                       |         |                   | 15/104.93        | EP 1007784 B1 2/2003                     |
| 2016/0160448 A1       | 6/2016  | Miller, IV et al. |                  | EP 1145695 A3 1/2004                     |
| 2016/0219810 A1       | 8/2016  | Erkkilä et al.    |                  | EP 1194644 B1 3/2004                     |
| 2016/0353820 A1       | 12/2016 | Baychar           |                  | EP 1457590 A1* 9/2004 D01F 6/34          |
| 2017/0016149 A1*      | 1/2017  | Nakamura .....    | D21H 15/02       | EP 1400224 B1 3/2006                     |

| (56)                     | References Cited |     |         |    |               |                  |
|--------------------------|------------------|-----|---------|----|---------------|------------------|
| FOREIGN PATENT DOCUMENTS |                  |     |         |    |               |                  |
| EP                       | 1384457          | B1  | 5/2006  | KR | 100685522     | B1               |
| EP                       | 1808116          | A1  | 7/2007  | KR | 100725240     | B1               |
| EP                       | 1649094          | B1  | 9/2007  | KR | 1020100112299 | A                |
| EP                       | 1442173          | B1  | 3/2008  | RU | 2393093       | C2               |
| EP                       | 1583865          | B1  | 5/2008  | SE | 7304825       | L                |
| EP                       | 1463432          | B1  | 8/2008  | SE | 7304888       | L                |
| EP                       | 1576233          | B1  | 10/2008 | SE | 412881        | B                |
| EP                       | 1813237          | A3  | 12/2008 | SE | 1651412       | A1               |
| EP                       | 1932968          | B1  | 9/2009  | SE | 540719        | C2               |
| EP                       | 1967626          | A4  | 9/2009  | WO | 1986003505    | A1               |
| EP                       | 1666240          | B1  | 3/2011  | WO | 1992003283    | A1               |
| EP                       | 1440195          | B1  | 8/2011  | WO | 9314267       | A1               |
| EP                       | 1812637          | B1  | 1/2012  | WO | 1996031652    | A1               |
| EP                       | 1950343          | B1  | 4/2012  | WO | 2000001882    | A1               |
| EP                       | 1456472          | B2  | 5/2012  | WO | 0025716       | A1               |
| EP                       | 1497489          | B1  | 8/2012  | WO | 2000050694    | A1               |
| EP                       | 1808152          | B1  | 8/2012  | WO | 0112902       | A1               |
| EP                       | 1567718          | B1  | 4/2013  | WO | 2001068793    | A1               |
| EP                       | 2599915          | A1  | 6/2013  | WO | 2001083866    | A2               |
| EP                       | 1268937          | B1  | 2/2014  | WO | 2002055788    | A2               |
| EP                       | 2540892          | B1  | 4/2014  | WO | 2003069038    | A1               |
| EP                       | 1876291          | B1  | 9/2014  | WO | 2004025009    | A2               |
| EP                       | 2843130          | A1  | 3/2015  | WO | 2004112956    | A1               |
| EP                       | 2952164          | A1  | 12/2015 | WO | 2005060712    | A2               |
| EP                       | 2952165          | A1  | 12/2015 | WO | 2006052967    | A2               |
| EP                       | 2737131          | B1  | 1/2016  | WO | 2006094077    | A2               |
| EP                       | 1916333          | B1  | 6/2016  | WO | 2007074625    | A1               |
| EP                       | 2001662          | B1  | 6/2016  | WO | 2009006371    | A2               |
| EP                       | 1380401          | B1  | 7/2016  | WO | 2009060118    | A2               |
| EP                       | 2807212          | B1  | 4/2017  | WO | 2011104427    | A1               |
| EP                       | 2940210          | B1  | 8/2017  | WO | 2014068196    | A2               |
| EP                       | 2622132          | B1  | 4/2018  | WO | 2014080084    | A1               |
| EP                       | 3327395          | A1  | 5/2018  | WO | 2014205048    | A1               |
| EP                       | 3162956          | B1  | 3/2019  | WO | 2015083092    | A1               |
| EP                       | 3108060          | B1  | 4/2021  | WO | 2015112155    | A1               |
| ES                       | 385106           | A1  | 3/1973  | WO | 2015173474    | A1               |
| ES                       | 8606100          | A1  | 4/1986  | WO | 2016050901    | A1               |
| ES                       | 2362723          | T3  | 7/2011  | WO | 2016051350    | A1               |
| FI                       | 812601           | A   | 2/1982  | WO | 16122477      | A1               |
| FI                       | 843904           | A   | 10/1984 | WO | 2016185398    | A1               |
| FI                       | 83741            | C   | 12/1992 | WO | 2016200299    | A1               |
| FI                       | 112812           | B   | 1/2004  | WO | 2017006216    | A1               |
| FI                       | 127377           | B   | 4/2018  | WO | 2017006241    | A1               |
| FI                       | 128917           | B   | 3/2021  | WO | 2017046751    | A1               |
| FR                       | 873763           | A   | 7/1942  | WO | 2017079169    | A1               |
| FR                       | 1449737          | A   | 8/1966  | WO | 2017137879    | A1               |
| FR                       | 1528992          | A   | 6/1968  | WO | 2018002815    | A1               |
| FR                       | 2206398          | B3  | 9/1976  | WO | 2018011667    | A1               |
| GB                       | 1145484          | A   | 3/1969  | WO | 2018041355    | A1               |
| GB                       | 2109023          | A   | 5/1983  | WO | 2018065668    | A1               |
| GB                       | 2136813          | A   | 9/1984  | WO | 2018116223    | A1               |
| GB                       | 2116882          | B   | 10/1985 | WO | 2018152082    | A1               |
| GB                       | 2582508          | A * | 9/2020  | WO | 2018171913    | A1               |
| IN                       | 1182DEL2005      | A   | 1/2007  | WO | 2018171914    | A1               |
| IN                       | 231170           | B   | 3/2009  | WO | WO-2018199975 | A1 *             |
| IN                       | 2957KOLNP2014    | A   | 5/2015  | WO | 11/2018       | ..... D21H 21/22 |
| IN                       | 3108MUM2014      | A   | 4/2016  | WO | WO-2019108172 | A1 *             |
| IN                       | 283291           | B   | 5/2017  | WO | 6/2019        | ..... D04H 1/559 |
| IN                       | 201717030330     | A   | 12/2017 |    |               |                  |
| IN                       | 201837033267     | A   | 10/2018 |    |               |                  |
| JP                       | 1983115199       | A   | 7/1983  |    |               |                  |
| JP                       | 1989501859       | A   | 6/1989  |    |               |                  |
| JP                       | 1993140886       | A   | 6/1993  |    |               |                  |
| JP                       | 4817935          | B2  | 11/2011 |    |               |                  |
| KR                       | 1020040088545    | A   | 10/2004 |    |               |                  |
| KR                       | 100450272        | B1  | 12/2005 |    |               |                  |
| KR                       | 100637646        | B1  | 10/2006 |    |               |                  |

## OTHER PUBLICATIONS

Vinda Paper (China) Co., Ltd, "Unbreakable in Water 3-layer Thickness Facial Tissue Paper", Jun. 16, 2017, <http://vinda.gmc.globalmarket.com/products/details/unbreakable-in-water-3-layer-thickness-facial-tissue-paper-10750223.html>.

\* cited by examiner



FIG. 1

EFFECT OF LAYERED VS. NON-LAYERED ON WET/DRY GMM RATIO



FIG. 2

**1**  
**FIBROUS SHEET WITH IMPROVED  
PROPERTIES**

BACKGROUND

Many tissue products, such as facial tissue, bath tissue, paper towels, industrial wipers, and the like, are produced according to a wet laid process. Wet laid webs are made by depositing an aqueous suspension of pulp fibers onto a forming fabric and then removing water from the newly-formed web. Water is typically removed from the web by mechanically pressing water out of the web that is referred to as "wet-pressing." Although wet-pressing is an effective dewatering process, during the process the tissue web is compressed causing a marked reduction in the caliper of the web and in the bulk of the web.

For most applications, however, it is desirable to provide the final product with as strength as possible without compromising other product attributes. Thus, those skilled in the art have devised various processes and techniques in order to increase the strength of wet laid webs. One process used is known as "rush transfer." During a rush transfer process, a web is transferred from a first moving fabric to a second moving fabric in which the second fabric is moving at a slower speed than the first fabric. Rush transfer processes increase the bulk, caliper, and softness of the tissue web.

As an alternative to wet-pressing processes, through-drying processes have developed in which web compression is avoided as much as possible to preserve and enhance the web. These processes provide for supporting the web on a coarse mesh fabric while heated air is passed through the web to remove moisture and dry the web.

Additional improvements in the art, however, are still needed. In particular, a need currently exists for an improved process that includes unique fibers in a tissue web for increasing the bulk, softness, strength, and absorbency of the web without having to subject the web to a rush transfer process or to a creping process.

SUMMARY

In general, the present disclosure is directed to further improvements in the art of tissue and papermaking. Through the processes and methods of the present disclosure, the properties of a tissue web, such as bulk, strength, stretch, caliper, and/or absorbency can be improved. In particular, the present disclosure is directed to a process for forming a nonwoven web, particularly a tissue web containing pulp fibers, in a foam-forming process. For example, a foam suspension of fibers can be formed and spread onto a moving porous conveyor for producing an embryonic web.

In one aspect, for instance, the present disclosure is directed to a method for producing a foam-formed multilayered substrate that includes producing an aqueous-based foam including at least 3% by weight non-straight synthetic binder fibers, wherein the non-straight synthetic binder fibers have an average length greater than 2 mm; forming together a wet sheet layer from the aqueous-based foam and a cellulosic fiber layer, wherein the cellulosic fiber layer includes at least 60 percent by weight cellulosic fibers; and drying the combined layers to obtain the foam-formed multilayer substrate.

In another aspect, a multilayered substrate includes a first layer including at least 60 percent by weight non-straight synthetic binder fibers having an average length greater than 2 mm; and a second layer including at least 60 percent by weight cellulosic fiber, wherein the first layer is in a facing

relationship with the second layer, and wherein the multilayered substrate has a wet/dry tensile ratio of at least 60%.

In yet another aspect, a multilayered substrate includes a first layer including at least 60 percent by weight non-straight synthetic binder fibers having an average length greater than 2 mm, wherein the non-straight synthetic binder fibers have a three-dimensional curly or crimped structure and are sheath-core bi-component fibers; and a second layer including at least 60 percent by weight cellulosic fiber, wherein the first layer is in a facing relationship with the second layer, wherein the multilayered substrate has a wet/dry tensile ratio of at least 60%, and wherein the multilayered substrate exhibits higher softness and absorbency than a homogeneous fibrous substrate with the same fiber composition.

Other features and aspects of the present disclosure are discussed in greater detail below.

BRIEF DESCRIPTION OF THE DRAWINGS

The foregoing and other features and aspects of the present disclosure and the manner of attaining them will become more apparent, and the disclosure itself will be better understood by reference to the following description, appended claims and accompanying drawings, where:

FIG. 1 is a schematic illustration of a foam-formed wet sheet being transferred from a forming wire onto a drying wire on a simplified tissue line; and

FIG. 2 is a graphic illustration comparing the effect of layered versus non-layered substrates on wet/dry geometric mean tensile (GMT) ratio.

Repeat use of reference characters in the present specification and drawings is intended to represent the same or analogous features or elements of the present disclosure. The drawings are representational and are not necessarily drawn to scale. Certain proportions thereof might be exaggerated, while others might be minimized.

DETAILED DESCRIPTION

It is to be understood by one of ordinary skill in the art that the present disclosure is a description of exemplary aspects of the present disclosure only, and is not intended as limiting the broader aspects of the present disclosure.

In general, the present disclosure is directed to the formation of tissue or paper webs having good bulk, strength, absorbency, and softness properties. Through the process of the present disclosure, tissue webs can be formed, for instance, having better stretch properties, improved absorbency characteristics, increased caliper, and/or increased softness. In one aspect, patterned webs can also be formed. In another aspect, for instance, a tissue web is made according to the present disclosure including the use of a foamed suspension of fibers.

High wet strength is important in towel products to have enough strength to hold together during hand drying or wiping up moisture. Standard towel sheets strive to have a wet/dry tensile of about 40% to have enough wet strength to work successfully. To achieve this level of wet strength in towels, refining and wet and dry strength chemistries are used.

The foam forming process opens up the opportunity to be able to add non-traditional fibers into the tissue making process. Fibers that normally would stay bundled together in the conventional wet laid process, such as longer length synthetic fibers, are now suspended and separated individually by foam bubbles, allowing the foam forming process to

offer not only the capability to make novel materials with non-standard wet-laid fibers but also basesheets with enhanced properties. Further, foam forming allows the use of non-straight synthetic binder fibers.

As used herein, "non-straight" synthetic binder fibers include synthetic binder fibers (described below) that are curved, sinusoidal, wavy, short waved, U-shaped, V-shaped where the angle is greater than 15° but less than 180°, bent, folded, crimped, crinkled, twisted, pucker, flagged, double flagged, randomly flagged, defined flagged, undefined flagged, split, double split, multi-prong tipped, double multi-prong tipped, hooked, interlocking, cone shaped, symmetrical, asymmetrical, fingered, textured, spiraled, looped, leaf-like, petal-like, or thorn-like. Long non-straight fibers have advantages described herein, but can be difficult to employ in a typical wet-laid process that usually only employs wood pulp cellulosic fiber having a fiber length less than 5 mm and typically less than 3 mm. One example of a suitable non-straight synthetic binder fiber is T-255 synthetic binder fiber available from Trevira. T-255 synthetic binder fiber is a non-straight and crimped bi-component fiber with a polyethylene terephthalate (PET) core and a polyethylene (PE) sheath.

There are many advantages and benefits to a foam-forming process as described above. During a foam-forming process, water is replaced with foam (i.e., air bubbles) as the carrier for the fibers that form the web. The foam, which represents a large quantity of air, is blended with papermaking fibers. Because less water is used to form the web, less energy is required to dry the web. For instance, drying the web in a foam-forming process can reduce energy requirements by greater than about 10%, or such as greater than about 20%, in relation to conventional wet pressing processes.

Foam-forming technology has proven its capabilities in bringing many benefits to products including improved fiber uniformity, reduced water amount in the process, reduced drying energy due to both reduced water amount and surface tension, improved capability of handling an extremely long or short fiber that enables an introduction of long staple and/or binder fibers and very short fiber fine into a regular wet laying process, and enhanced bulk/reduced density that broadens one process to be able to produce various materials from a high to a very low density to cover multiple product applications.

Bench experimentation using a high speed mixer and surfactant has produced a very low density, between 0.008 to 0.02 g/cc, foam-formed fibrous materials. Based on these results, an air-formed, 3D-structured, nonwoven-like fibrous material can be produced using a low cost but high speed wet laying process. Previous attempts to produce such low density fibrous materials using typical foam-forming lines did not produce favorable results. Both processes have equipment limitations preventing production of a low density or high bulk foam-formed fibrous material. One process lacks a drying capability and therefore must use a press with high pressure to remove water from a formed wet sheet as much as possible to gain wet sheet integrity, so the sheet can be wound onto a roll. In addition, another process does not have a pressure roll but has a continuous drying tunnel. While the latter process appears to have a potential to produce a low density fibrous material, the foam-formed wet sheet must be transferred from a forming fabric to a drying metal wire before it is dried inside the drying tunnel. Again, to gain enough wet sheet integrity for this transfer, the foam-formed sheet must be dewatered as much as possible by vacuum prior to this transfer. As a result, most of

entrapped air bubbles inside the wet sheet are also removed by the vacuum, resulting in a final dried sheet with a density similar to that of a sheet produced by a normal wet laying process.

5 Further experimentation resulted in the discovery that an addition of non-straight synthetic binder fibers reduces the final fibrous sheet density.

Without committing to a theory, it is believed that the non-straight synthetic binder fibers in a layered structure 10 help to achieve a high wet/dry tensile ratio. Prior art uses of crimped (non-binder) fibers had the goal of achieving high bulk. The non-straight synthetic binder fiber of the present disclosure would not work well to achieve high bulk. Whereas the prior art required a crimped (non-binder) fiber 15 having a fiber diameter at least 4 dtex, the non-straight synthetic binder fibers of the present disclosure do not have such a requirement. For example, one of the non-straight synthetic binder fibers used in the examples described below has a fiber diameter of 2.2 dtex.

20 According to the present disclosure, the foam-forming process is combined with a unique fiber addition for producing webs having a desired balance of properties.

In forming tissue or paper webs in accordance with the present disclosure, in one aspect, a foam is first formed by 25 combining water with a foaming agent. The foaming agent, for instance, can include any suitable surfactant. In one aspect, for instance, the foaming agent can include an anionic surfactant such as sodium lauryl sulfate, which is also known as sodium laureth sulfate and sodium lauryl ether sulfate. Other anionic foaming agents include sodium 30 dodecyl sulfate or ammonium lauryl sulfate. In other aspects, the foaming agent can include any suitable cationic, non-ionic, and/or amphoteric surfactant. For instance, other foaming agents include fatty acid amines, amides, amine 35 oxides, fatty acid quaternary compounds, polyvinyl alcohol, polyethylene glycol alkyl ether, polyoxyethylene sorbitan alkyl esters, glucoside alkyl ethers, cocamidopropyl hydroxysultaine, cocamidopropyl betaine, phosphatidylethanolamine, and the like.

40 The foaming agent is combined with water generally in an amount greater than about 0.001% by weight, such as in an amount greater than about 0.005% by weight, such as in an amount greater than about 0.01% by weight, or such as in an amount greater than about 0.05% by weight. The foaming 45 agent can also be combined with water generally in an amount less than about 0.2% by weight, such as in an amount less than about 0.5% by weight, such as in an amount less than about 1.0% by weight, or such as in an amount less than about 5% by weight. One or more foaming 50 agents are generally present in an amount less than about 5% by weight, such as in an amount less than about 2% by weight, such as in an amount less than about 1% by weight, or such as in an amount less than about 0.5% by weight.

Once the foaming agent and water are combined, the 55 mixture is combined with non-straight synthetic binder fibers. In general, any non-straight synthetic binder fibers capable of making a tissue or paper web or other similar type of nonwoven in accordance with the present disclosure can be used.

60 A binder fiber can be used in the foam formed fibrous structure of this disclosure. A binder fiber can be either a thermoplastic bicomponent fiber, such as PE/PET core/sheath fiber, or a water sensitive polymer fiber, such as polyvinyl alcohol fiber. Commercial binder fiber is usually 65 a bicomponent thermoplastic fiber with two different melting polymers. Two polymers used in this bicomponent fiber usually have quite different melting points. For example, a

PE/PET bicomponent fiber has a melting point of 120° C. for PE and a melting point of 260° C. for PET. When this bicomponent fiber is used as a binder fiber, a foam-formed fibrous structure including the PE/PET fiber can be stabilized by exposure to a heat treatment at a temperature slightly above 120° C. so that the PE fiber portion will melt and form inter-fiber bonds with other fibers while the PET fiber portion deliver its mechanical strength to maintain the fiber network intact. The bicomponent fiber can have different shapes with its two polymer components, such as, side-side, core-sheath, eccentric core-sheath, islands in a sea, etc. The core-sheath structure is the most commonly used in commercial binder fiber applications. Commercial binder fibers include T-255 binder fiber with a 6 or 12 mm fiber length and a 2.2 dtex fiber diameter from Trevira or WL Adhesion C binder fiber with a 4 mm fiber length and a 1.7 dtex fiber diameter from FiberVisions. The threshold amount of binder fiber to be added is generally dependent on the minimum that percolation theory would predict will provide a fiber network. For example, the percolation threshold is around 3% (by mass) for 6 mm, 2.2 dtex, T-255 fibers.

Once the foaming agent, water, and fibers are combined, the mixture is blended or otherwise subjected to forces capable of forming a foam. A foam generally refers to a porous matrix, which is an aggregate of hollow cells or bubbles that can be interconnected to form channels or capillaries.

The foam density can vary depending upon the particular application and various factors including the fiber furnish used. In one aspect, for instance, the foam density of the foam can be greater than about 200 g/L, such as greater than about 250 g/L, or such as greater than about 300 g/L. The foam density is generally less than about 600 g/L, such as less than about 500 g/L, such as less than about 400 g/L, or such as less than about 350 g/L. In one aspect, for instance, a lower density foam is used having a foam density of generally less than about 350 g/L, such as less than about 340 g/L, or such as less than about 330 g/L. The foam will generally have an air content of greater than about 40%, such as greater than about 50%, or such as greater than about 60%. The air content is generally less than about 80% by volume, such as less than about 75% by volume, or such as less than about 70% by volume.

To form the web, the foam is combined with a selected fiber furnish in conjunction with any auxiliary agents. The foam can be formed by any suitable method, including that described in co-pending U.S. Provisional Patent Application Ser. No. 62/437,974.

In general, any process capable of forming a paper web can also be utilized in the present disclosure. For example, a papermaking process of the present disclosure can utilize creping, double creping, embossing, air pressing, creped through-air drying, uncreped through-air drying, coform, hydroentangling, as well as other steps known in the art.

A standard process includes a foam-forming line that is designed to handle long staple fiber and is capable of achieving very uniform fiber mixing with other components. It is not, however, designed for producing high bulk fibrous material due to its equipment limitations as discussed above. FIG. 1 illustrates a simplified tissue line and demonstrates the difficulty in using this process to produce synthetic fibrous material, where a sheet is transferred between two wires. In this line, a frothed fibrous material or wet sheet 20 is formed onto a forming wire 30 by a headbox 35, where the wet sheet 20 has three layers of different compositions of fibrous materials when it is just laid onto the forming wire 30. The wet sheet 20 is then subjected to a vacuum to

remove as much of water as possible so that when the wet sheet 20 travels to the end of the first forming wire 30, it gains enough integrity or strength to allow the wet sheet 20 to be transferred to a drying wire 40.

There is a contacting point 50 between the forming and drying wires 30, 40 where the wet sheet 20 is transferred from the forming wire 30 and to the drying wire 40. After the wet sheet 20 is transferred to the drying wire 40, the wet sheet 20 keeps contact with but can fall from the drying wire 40 if the wet sheet 20 does not have sufficient amount of adhesion to overcome gravity. After the transfer, the wet sheet 20 is positioned underneath the drying wire 40. The wet sheet 20 needs to be adhered to the drying wire 40 before it reaches a through-air dried (TAD) dryer or other suitable dryer (not shown). When a wet sheet 20 contains majority of cellulosic fiber, the wet sheet 20 has a water absorption capability to keep water sufficient enough so that the wet sheet 20 adheres to the drying wire 40 without being fallen off the drying wire 40 by gravity. When a wet sheet 20 contains too much synthetic fiber, such as greater than 30%, the wet sheet 20 starts to fall or separate off the drying wire 40 due to gravity. In this method, the wet sheet 20 when containing more than 30% synthetic fiber did not have sufficient adhesion to keep the sheet attached to the drying wire 40 shown in FIG. 1.

Therefore, current processes prevent the production of any frothed material with more than 30% synthetic fibers. As a result, a modified process or a new fibrous composition is needed to produce a foam formed sheet with a high wet/dry tensile ratio. The present disclosure addresses this shortfall by forming a layered wet sheet 20 with two outer layers including a majority of cellulosic fiber and a center layer including a majority of synthetic binder fiber. This improved method overcomes the weak wire adhesion issue and at the same time achieves several benefits. First, binder fiber can be concentrated to almost 100% in the center layer to form a fully-bonded fiber network to achieve a high strength while keep overall synthetic fiber portion below 50%, or even below 30%, such that the final tissue remains cellulosic fiber based. A non-layered structure cannot achieve this. Second, the layered structure creates a non-uniform bonding point distribution. Most of the bonds are formed within the center layer among the binder fibers themselves with only slight bonding among the cellulosic fibers located in two outer layers. This arrangement allows the tissue to exhibit a high strength, high wet/dry tensile ratio, high bulk, high absorbency, and significantly enhanced overall softness.

All tissue sheets described herein are manufactured in un-creped through-air dried (UCTAD) mode. The UCTAD process uses vacuum to transfer the wet sheet from one fabric to another, as illustrated in FIG. 1. Learnings from previous foam forming trials have shown that adding more than about 30% synthetic fiber in a homogeneous sheet affects the ability of the sheet to transfer. This is due to insufficient water in the sheet for the vacuum to work. In the present disclosure this shortcoming was solved by making a multilayered substrate with cellulosic fibers for one or more outer layers using conventional wet-laid process parameters (pulp slurry run from machine chests using standard pumps and settings), with the center layer foam formed (run from dump chests where the foam slurry of non-straight synthetic binder fiber was generated by adding surfactant and mixed). The refined cellulose outer layers, because refined fibers hold more water, hold enough water to allow the sheet to be transferred. For this disclosure, a layer with up to 80% non-straight synthetic binder fibers was foam formed for the center layer.

In various aspects of the present disclosure, a multilayered substrate can include one cellulosic fiber outer layer (by wetlaid or other process) and one foam formed synthetic binder fiber middle layer, or two cellulosic fiber outer layers (by wetlaid or other process) and one foam formed synthetic binder fiber middle layer. The one or two outer layers can also be foam formed and also contain low percentage amount of synthetic fiber if additional benefits can be obtained. Preferred aspects include at least one layer that is foam formed and includes a high percentage of synthetic binder fiber to give the multilayered substrate a high wet/dry tensile ratio. Preferred aspects also include at least one outer layer that maintains direct contact with the drying wire 40 after sheet transfer, where that at least one outer layer includes a high percentage of cellulosic fiber to have sufficient sheet-wire adhesion during processing. Other layers added to the multilayered substrate can have any combination of foam formed and wetlaid layers and can include any amount of cellulosic and/or synthetic fibers.

One or more layers of a multilayered substrate can include cellulosic fibers including those used in standard tissue making. Fibers suitable for making tissue webs include any natural and/or synthetic cellulosic fibers. Natural fibers can include, but are not limited to, nonwoody fibers such as cotton, abaca, kenaf, sabai grass, flax, esparto grass, straw, jute hemp, bagasse, milkweed floss fibers, bamboo fibers, and pineapple leaf fibers; and woody or pulp fibers such as those obtained from deciduous and coniferous trees, including softwood fibers, such as northern and southern softwood kraft fibers; and hardwood fibers, such as *eucalyptus*, maple, birch, and aspen. Pulp fibers can be prepared in high-yield or low-yield forms and can be pulped in any known method, including kraft, sulfite, high-yield pulping methods, and other known pulping methods. Fibers prepared from organo-solv pulping methods can also be used.

A portion of the fibers, such as up to 50% or less by dry weight, or from about 5% to about 30% by dry weight, can be synthetic fibers. Regenerated or modified cellulose fiber types include rayon in all its varieties and other fibers derived from viscose or chemically-modified cellulose. Chemically-treated natural cellulosic fibers can be used such as mercerized pulps, chemically stiffened or crosslinked fibers, or sulfonated fibers. For good mechanical properties in using papermaking fibers, it can be desirable that the fibers be relatively undamaged and largely unrefined or only lightly refined. While recycled fibers can be used, virgin fibers are generally useful for their mechanical properties and lack of contaminants. Mercerized fibers, regenerated cellulosic fibers, cellulose produced by microbes, rayon, and other cellulosic material or cellulosic derivatives can be used. Suitable papermaking fibers can also include recycled fibers, virgin fibers, or mixes thereof. In certain aspects capable of high bulk and good compressive properties, the fibers can have a Canadian Standard Freeness of at least 200, more specifically at least 300, more specifically still at least 400, and most specifically at least 500.

Other papermaking fibers that can be used in the present disclosure include paper broke or recycled fibers and high yield fibers. High yield pulp fibers are those papermaking fibers produced by pulping processes providing a yield of about 65% or greater, more specifically about 75% or greater, and still more specifically about 75% to about 95%. Yield is the resulting amount of processed fibers expressed as a percentage of the initial wood mass. Such pulping processes include bleached chemithermomechanical pulp (BCTMP), chemithermomechanical pulp (CTMP), pressure/pressure thermomechanical pulp (PIMP), thermomechanical

pulp (TMP), thermomechanical chemical pulp (TMCP), high yield sulfite pulps, and high yield kraft pulps, all of which leave the resulting fibers with high levels of lignin. High yield fibers are well known for their stiffness in both dry and wet states relative to typical chemically pulped fibers.

Other optional chemical additives can also be added to the aqueous papermaking furnish or to the formed embryonic web to impart additional benefits to the product and process.

10 The following materials are included as examples of additional chemicals that can be applied to the web. The chemicals are included as examples and are not intended to limit the scope of the disclosure. Such chemicals can be added at any point in the papermaking process.

15 Additional types of chemicals that can be added to the paper web include, but are not limited to, absorbency aids usually in the form of cationic, anionic, or non-ionic surfactants, humectants and plasticizers such as low molecular weight polyethylene glycols and polyhydroxy compounds 20 such as glycerin and propylene glycol. Materials that supply skin health benefits such as mineral oil, aloe extract, vitamin E, silicone, lotions in general, and the like can also be incorporated into the finished products.

In general, the products of the present disclosure can be 25 used in conjunction with any known materials and chemicals that are not antagonistic to its intended use. Examples of such materials include but are not limited to odor control agents, such as odor absorbents, activated carbon fibers and particles, baby powder, baking soda, chelating agents, zeolites, perfumes or other odor-masking agents, cyclodextrin 30 compounds, oxidizers, and the like. Superabsorbent particles can also be employed. Additional options include cationic dyes, optical brighteners, humectants, emollients, and the like.

35 The basis weight of tissue webs made in accordance with the present disclosure can vary depending upon the final product. For example, the process can be used to produce bath tissues, facial tissues, paper towels, industrial wipers, and the like. In general, the basis weight of the tissue 40 products can vary from about 6 gsm to about 120 gsm, or such as from about 10 gsm to about 90 gsm. For bath tissue and facial tissues, for instance, the basis weight can range from about 10 gsm to about 40 gsm. For paper towels, on the other hand, the basis weight can range from about 25 gsm to 45 about 80 gsm.

The tissue web bulk can also vary from about 3 cc/g to 50 about 30 cc/g, or such as from about 5 cc/g to 15 cc/g. The sheet "bulk" is calculated as the quotient of the caliper of a dry tissue sheet, expressed in microns, divided by the dry 55 basis weight, expressed in grams per square meter. The resulting sheet bulk is expressed in cubic centimeters per gram. More specifically, the caliper is measured as the total thickness of a stack of ten representative sheets and dividing the total thickness of the stack by ten, where each sheet within the stack is placed with the same side up. Caliper is 60 measured in accordance with TAPPI test method T411 om-89 "Thickness (caliper) of Paper, Paperboard, and Combined Board" with Note 3 for stacked sheets. The micrometer used for carrying out T411 om-89 is an Emveco 200-A Tissue Caliper Tester available from Emveco, Inc., Newberg, Oreg. The micrometer has a load of 2.00 kilo-Pascals (132 grams per square inch), a pressure foot area of 2500 square millimeters, a pressure foot diameter of 56.42 millimeters, a dwell time of 3 seconds and a lowering rate of 0.8 millimeters per second.

In multiple ply products, the basis weight of each tissue web present in the product can also vary. In general, the total

basis weight of a multiple ply product will generally be the same as indicated above, such as from about 15 gsm to about 120 gsm. Thus, the basis weight of each ply can be from about 10 gsm to about 60 gsm, or such as from about 20 gsm to about 40 gsm.

### EXAMPLES

For the present disclosure, basesheets were made using a standard three-layered headbox. This headbox structure allows both layered and homogeneous (all fibers types mixed together throughout the sheet) structures to be produced. Both sheet structures were made to support this disclosure.

Examples for the present disclosure include a layered sheet with 100% cellulose for the outer layers using conventional wet-laid process parameters (pulp slurry run from machine chests using standard pumps and settings). The center layer was foam formed, run from dump chests where the foam slurry of 100% T-255 synthetic binder fiber was generated by adding surfactant and mixed. A layer of up to 40% synthetic fiber was foam formed for the center layer.

The different tissue codes generated for this disclosure are described in Table 1, along with the properties each tissue code demonstrated.

TABLE 1

| Tissue Compositions and Properties |                |              |                         |                |               |                |         |                   |
|------------------------------------|----------------|--------------|-------------------------|----------------|---------------|----------------|---------|-------------------|
| Structure                          |                |              | Tissue Properties       |                |               |                |         |                   |
| Code                               | Layered formed | Foam         | Composition             |                | Caliper (mil) | Density (g/cc) | Dry GMT | Wet/dry GMT Ratio |
|                                    |                |              | Outer layers            | Middle layer   |               |                |         |                   |
| 1                                  | Y              | Middle layer | 30% Euc                 | 40% T-255 6 mm | TBD           | TBD            | 1821    | 0.99              |
| 2                                  | Y              | Middle layer | 40% Euc                 | 20% T-255 6 mm | TBD           | TBD            | 952     | 0.76              |
| 3                                  | Y              | Middle layer | 45% Euc                 | 10% T-255 6 mm | 39.9          | 0.039          | 399     | No reading        |
| 4                                  | N              | All layers   | 90% Euc, 10% T-255 6 mm |                | 40.4          | 0.039          | 462     | 0.29              |
| 5                                  | N              | All layers   | 80% Euc, 20% T-255 6 mm |                | 35.2          | 0.045          | 433     | 0.35              |

The basis weights were 40.5 gsm for Code 1, 42 gsm for Code 2, and 40 gsm for Codes 3-5. Euc is *eucalyptus*. Codes 2 and 5 show a direct comparison between layered and mixed substrates using the same overall fiber amounts.

GMT is geometric mean tensile strength that takes into account the machine direction (MD) tensile strength and the cross-machine direction (CD) tensile strength. For purposes herein, tensile strength can be measured using a SINTECH tensile tester using a 3-inch jaw width (sample width), a jaw span of 2 inches (gauge length), and a crosshead speed of 25.4 centimeters per minute after maintaining the sample under TAPPI conditions for 4 hours before testing. The "MD tensile strength" is the peak load per 3 inches of sample width when a sample is pulled to rupture in the machine direction. Similarly, the "CD tensile strength" represents the peak load per 3 inches of sample width when a sample is pulled to rupture in the cross-machine direction. The GMT is the square root of the product of the MD tensile strength and the CD tensile strength of the web. The "CD stretch" and the "MD stretch" are the amount of sample elongation in the cross-machine direction and the machine direction, respectively, at the point of rupture, expressed as a percent of the initial sample length.

More particularly, samples for tensile strength testing are prepared by cutting a 3 inch (76.2 mm) wide by at least 4 inches (101.6 mm) long strip in either the machine direction (MD) or cross-machine direction (CD) orientation using a JDC Precision Sample Cutter (Thwing-Albert Instrument Company, Philadelphia, Pa., Model No. JDC 3-10, Serial

No. 37333). The instrument used for measuring tensile strength is an MTS Systems SINTECH Serial No. 1G/071896/116. The data acquisition software is MTS TestWorks® for Windows Ver. 4.0 (MTS Systems Corp., Eden Prairie, Minn.). The load cell is an MTS 25 Newton maximum load cell. The gauge length between jaws is  $2\pm0.04$  inches ( $76.2\pm1$  mm). The jaws are operated using pneumatic action and are rubber coated. The minimum grip face width is 3 inches (76.2 mm), and the approximate height of a jaw is 0.5 inches (12.7 mm). The break sensitivity is set at 40 percent. The sample is placed in the jaws of the instrument, centered both vertically and horizontally. To adjust the initial slack, a pre-load of 1 gram (force) at the rate of 0.1 inch per minute is applied for each test run. The test is then started and ends when the force drops by 40 percent of peak. The peak load is recorded as either the "MD tensile strength" or the "CD tensile strength" of the specimen depending on the sample being tested. At least 3 representative specimens are tested for each product, taken "as is," and the arithmetic average of all individual specimen tests is either the MD or CD tensile strength for the product.

Beside the significantly-enhanced wet/dry tensile ratio demonstrated in Table 1, data also indicated that the layered UCTAD tissues listed in Table 1 exhibit improved softness and absorbency, as shown in Table 2.

The two control codes described in Table 2 consist of a homogeneous mixed fiber sheet containing 100% cellulose pulp fiber (UCTAD Bath CHF controls from January 2015-September 2016). PBS stands for Premium Bath Score and is derived from the formulation below consisting of several Sensory Panel tests performed on the tissue basesheet.

$$\text{PBS} = 5 * (\text{Average Fuzzy} + \text{Volume} - \text{Rigidity} - \text{Average Gritty}) + 25$$

The higher the PBS value, the softer the tissue is perceived to be. Table 2 demonstrates that layered structures, at the same strength, exhibit improved softness compared to homogeneous structures.

TABLE 2

| Perceived Tissue Softness |                    |          |     |
|---------------------------|--------------------|----------|-----|
| Code                      | Basis Weight (gsm) | GMT (gf) | PBS |
| 1*                        | 40.5               | 1272     | 64  |
| 2*                        | 42                 | 1054     | 64  |
| Control Code A            | 40                 | 1100     | 46  |
| Control Code B            | 40                 | 1300     | 41  |

Note:

\*Codes 1 and 2 are the same materials as Codes 1 and 2 in Table 1, except that Codes 1 and 2 in Table 2 have been calendered.

GMT is geometric mean tensile strength and is described above in more detail.

Codes 1 and 2 were manufactured as bath tissue. As demonstrated in Table 3, the Codes 1 and 2 bath tissue with

## 11

layered structures exhibited the same or slightly better absorbency than current commercial towel products. Towel products normally have higher absorbency than bath tissue. Absorption capacity is determined using a 4 inch by 4 inch specimen that is initially weighed. The weighed specimen is then soaked in a pan of test fluid (e.g. paraffin oil or water) for three minutes. The test fluid should be at least 2 inches (5.08 cm) deep in the pan. The specimen is removed from the test fluid and allowed to drain while hanging in a "diamond" shaped position (i.e., with one corner at the lowest point). The specimen is allowed to drain for three minutes for water and for five minutes for oil. After the allotted drain time the specimen is placed in a weighing dish and weighed. The absorbency of acids or bases having a viscosity more similar to water is tested in accordance with the procedure for testing the absorption capacity for water. Absorption Capacity (g)=wet weight (g)-dry weight (g); and Specific Absorption Capacity (g/g)=Absorption Capacity (g)/dry weight (g).

TABLE 3

| Absorbency Data as Specific Absorption Capacity in g/g |                                                                        |                                  |
|--------------------------------------------------------|------------------------------------------------------------------------|----------------------------------|
| Codes                                                  | Description                                                            | Specific Absorption Capacity g/g |
| BOUNTY<br>brand towels                                 | Commercial                                                             | 8.25                             |
| BRAWNY<br>brand towels                                 | Commercial                                                             | 9.06                             |
| VIVA<br>brand towels                                   | Commercial                                                             | 8.84                             |
| Code 1*                                                | CHF Layered <i>eucalyptus</i> 30%/<br>T-255 40%/ <i>eucalyptus</i> 30% | 9.27                             |
| Code 2*                                                | CHF Layered <i>eucalyptus</i> 40%/<br>T-255 20%/ <i>eucalyptus</i> 40% | 8.87                             |

## Note:

\*Codes 1 and 2 are the same materials as Codes 1 and 2 in Table 1, except that Codes 1 and 2 in Table 2 have been calendered.

It should be noted that while the examples in this disclosure were produced using a foam forming process, the disclosure should not be limited to such a process. The foam forming process is employed due to its capability of handling long fiber, such as 6 mm or 12 mm binder fiber. Conversely, if a short binder fiber (e.g., 2 mm or shorter) is used, the same layered structure can be produced using a standard water-forming process.

## Results

As demonstrated in Tables 1-3, the layered structure with two cellulose fiber rich outer layers and one non-straight synthetic binder fiber rich middle layer exhibits a significant enhancement in wet/dry tensile ratio when compared to a substrate having the same fiber composition but homogeneously mixed (i.e., a non-layered structure). This can be seen best in a comparison between Codes 2 and 5 in Table 1. Additional data is provided in FIG. 2, demonstrating the improvement in wet/dry tensile ratio in layered versus non-layered substrates having the same fiber compositions.

In a first particular aspect, a method for producing a foam-formed multilayered substrate includes producing an aqueous-based foam including at least 3% by weight non-straight synthetic binder fibers, wherein the non-straight synthetic binder fibers have an average length greater than 2 mm; forming together a wet sheet layer from the aqueous-based foam and a cellulosic fiber layer, wherein the cellulosic fiber layer includes at least 60 percent by weight

## 12

cellulosic fibers; and drying the combined layers to obtain the foam-formed multilayer substrate.

A second particular aspect includes the first particular aspect, wherein the foam-formed layer has a dry density between 0.008 g/cc and 0.1 g/cc.

A third particular aspect includes the first and/or second aspect, wherein the non-straight synthetic binder fibers have an average length from 4 mm to 60 mm.

A fourth particular aspect includes one or more of aspects 10 1-3, wherein the non-straight synthetic binder fibers have an average length from 6 mm to 30 mm.

A fifth particular aspect includes one or more of aspects 1-4, wherein the non-straight synthetic binder fibers have a diameter of at least 1.5 dtex.

15 A sixth particular aspect includes one or more of aspects 1-5, wherein the non-straight synthetic binder fibers have a three-dimensional curly structure.

A seventh particular aspect includes one or more of aspects 1-6, wherein the non-straight synthetic binder fibers 20 have a three-dimensional crimped structure.

An eighth particular aspect includes one or more of aspects 1-7, wherein the non-straight synthetic binder fibers are bi-component fibers.

A ninth particular aspect includes one or more of aspects 25 1-8, wherein the bi-component fibers are sheath-core bi-component fibers.

A tenth particular aspect includes one or more of aspects 1-9, wherein the sheath is polyethylene and the core is polyester.

30 An eleventh particular aspect includes one or more of aspects 1-10, wherein producing includes at least 10% by weight non-straight synthetic binder fibers.

A twelfth particular aspect includes one or more of aspects 1-11, wherein the multilayered substrate has a wet/dry tensile ratio of 60% or higher.

A thirteenth particular aspect includes one or more of aspects 1-12, wherein the cellulosic fibers are *eucalyptus* fibers.

35 In a fourteenth particular aspect, a multilayered substrate includes a first layer including at least 60 percent by weight non-straight synthetic binder fibers having an average length greater than 2 mm; and a second layer including at least 60 percent by weight cellulosic fiber, wherein the first layer is in a facing relationship with the second layer, and wherein 45 the multilayered substrate has a wet/dry tensile ratio of at least 60%.

A fifteenth particular aspect includes the fourteenth particular aspect, wherein the multilayered substrate exhibits higher softness and absorbency than a homogeneous fibrous substrate with the same fiber composition.

A sixteenth particular aspect includes the fourteenth and/or fifteenth aspect, wherein the non-straight synthetic binder fibers have an average length from 6 mm to 30 mm and an average diameter of at least 1.5 dtex.

55 A seventeenth particular aspect includes one or more of aspects 14-16, wherein the non-straight synthetic binder fibers have a three-dimensional curly or crimped structure.

An eighteenth particular aspect includes one or more of aspects 14-17, wherein the non-straight synthetic binder fibers are sheath-core bi-component fibers.

A nineteenth particular aspect includes one or more of aspects 14-18, wherein the sheath is polyethylene and the core is polyester.

60 In a twentieth particular aspect, a multilayered substrate includes a first layer including at least 60 percent by weight non-straight synthetic binder fibers having an average length greater than 2 mm, wherein the non-straight synthetic binder

## 13

fibers have a three-dimensional curly or crimped structure and are sheath-core bi-component fibers; and a second layer including at least 60 percent by weight cellulosic fiber, wherein the first layer is in a facing relationship with the second layer, wherein the multilayered substrate has a wet/dry tensile ratio of at least 60%, and wherein the multilayered substrate exhibits higher softness and absorbency than a homogeneous fibrous substrate with the same fiber composition.

These and other modifications and variations to the present disclosure can be practiced by those of ordinary skill in the art, without departing from the spirit and scope of the present disclosure, which is more particularly set forth in the appended claims. In addition, it should be understood that aspects of the various aspects of the present disclosure may be interchanged either in whole or in part. Furthermore, those of ordinary skill in the art will appreciate that the foregoing description is by way of example only, and is not intended to limit the disclosure so further described in such appended claims.

What is claimed is:

1. A method for producing a foam-formed multilayered substrate, the method comprising:  
 producing an aqueous-based foam including at least 3% by weight non-straight synthetic binder fibers, wherein the non-straight synthetic binder fibers have an average length greater than 2 mm;  
 forming combined layers by combining together a wet sheet layer from the aqueous-based foam and a cellulosic fiber layer, wherein the cellulosic fiber layer includes at least 60 percent by weight cellulosic fibers;  
 exposing the combined layers to heat such that at least a portion of the non-straight synthetic binder fibers melt to form inter-fiber bonds; and

## 14

drying the combined layers to obtain the foam-formed multilayer substrate.

2. The method of claim 1, wherein the wet sheet layer from the aqueous-based foam has a dry density between 0.008 g/cc and 0.1 g/cc.

3. The method of claim 1, wherein the non-straight synthetic binder fibers have an average length from 4 mm to 60 mm.

4. The method of claim 1, wherein the non-straight synthetic binder fibers have an average length from 6 mm to 30 mm.

5. The method of claim 1, wherein the non-straight synthetic binder fibers have a diameter of at least 1.5 dtex.

6. The method of claim 1, wherein the non-straight synthetic binder fibers have a three-dimensional curly structure.

7. The method of claim 1, wherein the non-straight synthetic binder fibers have a three-dimensional crimped structure.

8. The method of claim 1, wherein the non-straight synthetic binder fibers are bi-component fibers.

9. The method of claim 8, wherein the bi-component fibers are sheath-core bi-component fibers.

10. The method of claim 9, wherein the sheath is polyethylene and the core is polyester.

11. The method of claim 1, wherein producing includes at least 10% by weight non-straight synthetic binder fibers.

12. The method of claim 11, wherein the multilayered substrate has a wet/dry tensile ratio of 60% or higher.

13. The method of claim 12, wherein the foam-formed multilayered substrate is produced in an un-creped through-air dried mode.

14. The method of claim 1, wherein the cellulosic fibers are *eucalyptus* fibers.

\* \* \* \* \*